



US011952648B2

(12) **United States Patent**  
**Valdez et al.**

(10) **Patent No.:** **US 11,952,648 B2**  
(b4) **Date of Patent:** **Apr. 9, 2024**

(54) **METHOD OF FORMING AND HEAT TREATING COILED TUBING**

(71) Applicant: **TENARIS COILED TUBES, LLC**,  
Houston, TX (US)

(72) Inventors: **Martin Valdez**, Buenos Aires (AR);  
**Bruce A. Reichert**, Houston, TX (US);  
**Jorge Mitre**, Houston, TX (US)

(73) Assignee: **Tenaris Coiled Tubes, LLC**, Houston,  
TX (US)

(\*) Notice: Subject to any disclaimer, the term of this  
patent is extended or adjusted under 35  
U.S.C. 154(b) by 246 days.

(21) Appl. No.: **16/685,333**

(22) Filed: **Nov. 15, 2019**

(65) **Prior Publication Data**

US 2020/0102633 A1 Apr. 2, 2020

**Related U.S. Application Data**

(60) Continuation of application No. 14/872,490, filed on  
Oct. 1, 2015, now Pat. No. 10,480,054, which is a  
division of application No. 13/229,517, filed on Sep.  
9, 2011, now Pat. No. 9,163,296.

(60) Provisional application No. 61/436,156, filed on Jan.  
25, 2011.

(51) **Int. Cl.**

**C21D 9/10** (2006.01)  
**C21D 6/00** (2006.01)  
**C21D 8/10** (2006.01)  
**C21D 9/08** (2006.01)  
**C21D 9/14** (2006.01)  
**C22C 38/02** (2006.01)  
**C22C 38/04** (2006.01)  
**C22C 38/06** (2006.01)  
**C22C 38/26** (2006.01)  
**C22C 38/28** (2006.01)  
**C22C 38/32** (2006.01)  
**C22C 38/38** (2006.01)  
**E21B 17/20** (2006.01)

(52) **U.S. Cl.**

CPC ..... **C22C 38/38** (2013.01); **C21D 6/002**  
(2013.01); **C21D 6/005** (2013.01); **C21D  
6/008** (2013.01); **C21D 8/105** (2013.01);  
**C21D 9/08** (2013.01); **C21D 9/085** (2013.01);  
**C21D 9/14** (2013.01); **C22C 38/02** (2013.01);  
**C22C 38/04** (2013.01); **C22C 38/06** (2013.01);  
**C22C 38/26** (2013.01); **C22C 38/28** (2013.01);  
**C22C 38/32** (2013.01); **E21B 17/20** (2013.01)

(58) **Field of Classification Search**

CPC ..... C21D 6/002; C21D 6/005; C21D 6/008;  
C21D 8/105; C21D 9/08; C21D 9/085;  
C21D 9/14; C22C 38/02; C22C 38/04;  
C22C 38/06; C22C 38/26; C22C 38/28;  
C22C 38/32; C22C 38/38; E21B 17/20

See application file for complete search history.

(56)

**References Cited**

U.S. PATENT DOCUMENTS

3,316,395 A 4/1967 Lavin  
3,316,396 A 4/1967 Lavin  
3,325,174 A 6/1967 Weaver  
3,362,731 A 1/1968 Gasche et al.  
3,366,392 A 1/1968 Kennel  
3,413,166 A 11/1968 Zackay et al.  
3,489,437 A 1/1970 Duret  
3,512,789 A 5/1970 Tanner  
3,552,781 A 1/1971 Helland  
3,572,777 A 3/1971 Blose et al.  
3,575,430 A 4/1971 Alpine  
3,592,491 A 7/1971 Glover  
3,599,931 A 8/1971 Hanson  
3,655,465 A 4/1972 Snape et al.  
3,733,093 A 5/1973 Seiler  
3,810,793 A 5/1974 Heller  
3,854,760 A 12/1974 Duret  
3,889,989 A 6/1975 Legris et al.  
3,891,224 A 6/1975 Ditcher  
3,893,919 A 7/1975 Flegel et al.  
3,915,697 A 10/1975 Giuliani et al.  
3,918,726 A 11/1975 Kramer  
3,986,731 A 10/1976 De Hoff  
4,014,568 A 3/1977 Carter et al.  
4,147,368 A 4/1979 Baker et al.

(Continued)

FOREIGN PATENT DOCUMENTS

AR 0050159 10/2006  
AT 388791 B 8/1989

(Continued)

OTHER PUBLICATIONS

US SDTX; Civil Action No. 4:17-CV-03299 *Global Tubing LLC vs. Tenaris Coiled Tubes LLC, et al*; Order, Mar. 20, 2023.  
Thompson et al., "Full Body Quenched and Tempered Coiled Tubing—Theory vs. Field Experience," Presented at the Second  
(Continued)

Primary Examiner — Jenny R Wu

(74) Attorney, Agent, or Firm — Morgan, Lewis &  
Bockius LLP

(57)

**ABSTRACT**

Described herein are coiled tubes with improved and varying properties along the length that are produced by using a continuous and dynamic heat treatment process (CDHT). Coiled tubes can be uncoiled from a spool, subjected to a CDHT process, and coiled onto a spool. A CDHT process can produce a "composite" tube such that properties of the tube along the length of the tube are selectively varied. For example, the properties of the tube can be selectively tailored along the length of the tube for particular application for which the tube will be used.

(56)

## References Cited

## U.S. PATENT DOCUMENTS

|               |         |                   |              |         |                      |
|---------------|---------|-------------------|--------------|---------|----------------------|
| 4,163,290 A   | 7/1979  | Sutherlin et al.  | 5,879,474 A  | 3/1999  | Bhadeshia et al.     |
| 4,219,204 A   | 8/1980  | Pippert           | 5,944,921 A  | 8/1999  | Cumino et al.        |
| 4,231,555 A   | 11/1980 | Saito             | 5,993,570 A  | 11/1999 | Gray                 |
| 4,299,412 A   | 11/1981 | Parmann           | 6,006,789 A  | 12/1999 | Toyooka et al.       |
| 4,305,059 A   | 12/1981 | Benton            | 6,030,470 A  | 2/2000  | Hensger et al.       |
| 4,310,163 A   | 1/1982  | Pippert           | 6,044,539 A  | 4/2000  | Guzowksi             |
| 4,336,081 A   | 6/1982  | Hijikata et al.   | 6,045,165 A  | 4/2000  | Sugino et al.        |
| 4,345,739 A   | 8/1982  | Wheatley          | 6,056,324 A  | 5/2000  | Reimert et al.       |
| 4,354,882 A   | 10/1982 | Greer             | 6,070,912 A  | 6/2000  | Latham               |
| 4,366,971 A   | 1/1983  | Lula              | 6,173,968 B1 | 1/2001  | Nelson et al.        |
| 4,368,894 A   | 1/1983  | Parmann           | 6,188,037 B1 | 2/2001  | Hamada et al.        |
| 4,373,750 A   | 2/1983  | Mantelle et al.   | 6,196,530 B1 | 3/2001  | Muhr et al.          |
| 4,376,528 A   | 3/1983  | Ohshimatai et al. | 6,217,676 B1 | 4/2001  | Takabe et al.        |
| 4,379,482 A   | 4/1983  | Suzuki et al.     | 6,248,187 B1 | 6/2001  | Asahi et al.         |
| 4,384,737 A   | 5/1983  | Reusser           | 6,257,056 B1 | 7/2001  | Shibayama            |
| 4,406,561 A   | 9/1983  | Ewing             | 6,267,828 B1 | 7/2001  | Kushida et al.       |
| 4,407,681 A   | 10/1983 | Ina et al.        | 6,311,965 B1 | 11/2001 | Muhr et al.          |
| 4,426,095 A   | 1/1984  | Buttner           | 6,331,216 B1 | 12/2001 | Toyooka et al.       |
| 4,445,265 A   | 5/1984  | Olson et al.      | 6,347,814 B1 | 2/2002  | Cerruti              |
| 4,473,471 A   | 9/1984  | Robichaud et al.  | 6,349,979 B1 | 2/2002  | Noel et al.          |
| 4,475,839 A   | 10/1984 | Strandberg        | 6,358,336 B1 | 3/2002  | Miyata               |
| 4,491,725 A   | 1/1985  | Pritchard         | 6,384,388 B1 | 5/2002  | Anderson et al.      |
| 4,506,432 A   | 3/1985  | Smith             | 6,412,831 B1 | 7/2002  | Noel et al.          |
| 4,526,628 A   | 7/1985  | Ohno et al.       | 6,447,025 B1 | 9/2002  | Smith                |
| 4,527,815 A   | 7/1985  | Smith             | 6,478,344 B2 | 11/2002 | Pallini, Jr. et al.  |
| 4,564,392 A   | 1/1986  | Ohhashi et al.    | 6,481,760 B1 | 11/2002 | Noel et al.          |
| 4,570,982 A   | 2/1986  | Blose et al.      | 6,494,499 B1 | 12/2002 | Galle, Sr. et al.    |
| 4,591,195 A   | 5/1986  | Chelette et al.   | 6,514,359 B2 | 2/2003  | Kawano               |
| 4,592,558 A   | 6/1986  | Hopkins           | 6,527,056 B2 | 3/2003  | Newman               |
| 4,601,491 A   | 7/1986  | Bell, Jr. et al.  | 6,540,848 B2 | 4/2003  | Miyata et al.        |
| 4,602,807 A   | 7/1986  | Bowers            | 6,550,822 B2 | 4/2003  | Mannella et al.      |
| 4,623,173 A   | 11/1986 | Handa et al.      | 6,557,906 B1 | 5/2003  | Carcagno             |
| 4,629,218 A * | 12/1986 | Dubois .....      | 6,558,484 B1 | 5/2003  | Onoe et al.          |
|               |         | E21B 17/20        | 6,581,940 B2 | 6/2003  | Dittel               |
|               |         | 138/155           | 6,632,296 B2 | 10/2003 | Yoshinaga et al.     |
| 4,662,659 A   | 5/1987  | Blose et al.      | 6,648,991 B2 | 11/2003 | Turconi et al.       |
| 4,674,756 A   | 6/1987  | Fallon et al.     | 6,669,285 B1 | 12/2003 | Park et al.          |
| 4,688,832 A   | 8/1987  | Orloff et al.     | 6,669,789 B1 | 12/2003 | Edelman et al.       |
| 4,706,997 A   | 11/1987 | Carstensen        | 6,682,610 B1 | 1/2004  | Inoue                |
| 4,710,245 A   | 12/1987 | Roether           | 6,683,834 B2 | 1/2004  | Ohara et al.         |
| 4,721,536 A   | 1/1988  | Koch et al.       | 6,709,534 B2 | 3/2004  | Kusinski et al.      |
| 4,758,025 A   | 7/1988  | Frick             | 6,752,436 B1 | 6/2004  | Verdillon            |
| 4,762,344 A   | 8/1988  | Perkins et al.    | 6,755,447 B2 | 6/2004  | Galle, Jr. et al.    |
| 4,812,182 A   | 3/1989  | Fang et al.       | 6,764,108 B2 | 7/2004  | Ernst et al.         |
| 4,814,141 A   | 3/1989  | Imai et al.       | 6,767,417 B2 | 7/2004  | Fujita et al.        |
| 4,844,517 A   | 7/1989  | Beiley et al.     | 6,814,358 B2 | 11/2004 | Keck                 |
| 4,856,828 A   | 8/1989  | Kessler et al.    | 6,851,727 B2 | 2/2005  | Carcagno et al.      |
| 4,955,645 A   | 9/1990  | Weems             | 6,857,668 B2 | 2/2005  | Otten et al.         |
| 4,958,862 A   | 9/1990  | Cappelli et al.   | 6,883,804 B2 | 4/2005  | Cobb                 |
| 4,988,127 A   | 1/1991  | Cartensen         | 6,905,150 B2 | 6/2005  | Carcagno et al.      |
| 5,007,665 A   | 4/1991  | Bovisio et al.    | 6,921,110 B2 | 7/2005  | Marotti et al.       |
| 5,067,874 A   | 11/1991 | Foote             | 6,958,099 B2 | 10/2005 | Nakamura et al.      |
| 5,137,310 A   | 8/1992  | Noel et al.       | 6,971,681 B2 | 12/2005 | Dell'Erba et al.     |
| 5,143,381 A   | 9/1992  | Temple            | 6,991,267 B2 | 1/2006  | Ernst et al.         |
| 5,154,534 A   | 10/1992 | Guerin et al.     | 7,014,223 B2 | 3/2006  | Della Pina et al.    |
| 5,180,008 A   | 1/1993  | Aldridge et al.   | 7,066,499 B2 | 6/2006  | Della Pina et al.    |
| 5,191,911 A   | 3/1993  | Dubois            | 7,074,283 B2 | 7/2006  | Omura                |
| 5,242,199 A   | 9/1993  | Hann et al.       | 7,083,686 B2 | 8/2006  | Itou                 |
| 5,328,158 A   | 7/1994  | Lewis             | 7,108,063 B2 | 9/2006  | Carstensen           |
| 5,348,350 A   | 9/1994  | Blose et al.      | 7,118,637 B2 | 10/2006 | Kusinski et al.      |
| 5,352,406 A   | 10/1994 | Barteri et al.    | 7,182,140 B2 | 2/2007  | Wood                 |
| 5,360,239 A   | 11/1994 | Klementich        | 7,214,278 B2 | 5/2007  | Kusinski et al.      |
| 5,449,420 A   | 9/1995  | Okada et al.      | 7,255,374 B2 | 8/2007  | Carcagno et al.      |
| 5,454,883 A   | 10/1995 | Yoshie et al.     | 7,264,684 B2 | 9/2007  | Numata et al.        |
| 5,456,405 A   | 10/1995 | Stagg             | 7,284,770 B2 | 10/2007 | Dell'Erba et al.     |
| 5,505,502 A   | 4/1996  | Smith et al.      | 7,310,867 B2 | 12/2007 | Corbett, Jr.         |
| 5,515,707 A   | 5/1996  | Smith             | 7,431,347 B2 | 10/2008 | Ernst et al.         |
| 5,538,566 A   | 7/1996  | Gallagher         | 7,464,449 B2 | 12/2008 | Santi et al.         |
| 5,592,988 A   | 1/1997  | Meroni et al.     | 7,475,476 B2 | 1/2009  | Roussie              |
| 5,598,735 A   | 2/1997  | Saito et al.      | 7,478,842 B2 | 1/2009  | Reynolds, Jr. et al. |
| 5,653,452 A   | 8/1997  | Jarvenkyla        | 7,506,900 B2 | 3/2009  | Carcagno et al.      |
| 5,712,706 A   | 1/1998  | Castore et al.    | 7,621,034 B2 | 11/2009 | Roussie              |
| 5,794,985 A   | 8/1998  | Mallis            | 7,635,406 B2 | 12/2009 | Numata et al.        |
| 5,810,401 A   | 9/1998  | Mosing et al.     | 7,735,879 B2 | 6/2010  | Toscano et al.       |
| 5,860,680 A   | 1/1999  | Drijver et al.    | 7,744,708 B2 | 6/2010  | Lopez et al.         |
| 5,879,030 A   | 3/1999  | Clayson et al.    | 7,753,416 B2 | 7/2010  | Mazzaferro et al.    |
|               |         |                   | 7,862,667 B2 | 1/2011  | Turconi et al.       |
|               |         |                   | 8,002,910 B2 | 8/2011  | Tivelli et al.       |
|               |         |                   | 8,007,601 B2 | 8/2011  | Lopez et al.         |

| (56)                  | References Cited |                      |                          |           |                   |         |  |
|-----------------------|------------------|----------------------|--------------------------|-----------|-------------------|---------|--|
| U.S. PATENT DOCUMENTS |                  |                      |                          |           |                   |         |  |
| 8,007,603 B2          | 8/2011           | Garcia et al.        | 2008/0314481 A1          | 12/2008   | Garcia et al.     |         |  |
| 8,016,362 B2          | 9/2011           | Itoga                | 2009/0010794 A1          | 1/2009    | Turconi et al.    |         |  |
| 8,262,094 B2          | 9/2012           | Beele                | 2009/0033087 A1          | 2/2009    | Carcagno et al.   |         |  |
| 8,262,140 B2          | 9/2012           | Santi et al.         | 2009/0047166 A1          | 2/2009    | Tomomatsu et al.  |         |  |
| 8,317,946 B2          | 11/2012          | Arai et al.          | 2009/0101242 A1          | 4/2009    | Lopez et al.      |         |  |
| 8,328,958 B2          | 12/2012          | Turconi et al.       | 2009/0114318 A1          | 5/2009    | Arai et al.       |         |  |
| 8,328,960 B2          | 12/2012          | Gomez et al.         | 2009/0148334 A1          | 6/2009    | Stephenson        |         |  |
| 8,333,409 B2          | 12/2012          | Santi et al.         | 2009/0226491 A1          | 9/2009    | Satou et al.      |         |  |
| 8,414,715 B2          | 4/2013           | Altschuler et al.    | 2009/0226988 A1          | 9/2009    | Tajima et al.     |         |  |
| 8,544,304 B2          | 10/2013          | Santi                | 2010/0136363 A1          | 6/2010    | Valdez et al.     |         |  |
| 8,821,653 B2          | 9/2014           | Anelli et al.        | 2010/0187808 A1          | 7/2010    | Santi             |         |  |
| 8,840,152 B2          | 9/2014           | Carcagno et al.      | 2010/0193085 A1          | 8/2010    | Garcia            |         |  |
| 8,926,771 B2          | 1/2015           | Agazzi               | 2010/0206553 A1          | 8/2010    | Bailey et al.     |         |  |
| 9,004,544 B2          | 4/2015           | Carcagno et al.      | 2010/0294401 A1          | 11/2010   | Gomez             |         |  |
| 9,163,296 B2          | 10/2015          | Valdez et al.        | 2010/0319814 A1          | 12/2010   | Perez             |         |  |
| 9,187,811 B2          | 11/2015          | Gomez et al.         | 2010/0327550 A1          | 12/2010   | Lopez             |         |  |
| 9,222,156 B2          | 12/2015          | Altschuler et al.    | 2011/0042946 A1          | 2/2011    | Santi             |         |  |
| 9,234,612 B2          | 1/2016           | Santi et al.         | 2011/0077089 A1          | 3/2011    | Hirai et al.      |         |  |
| 9,340,847 B2          | 5/2016           | Altschuler et al.    | 2011/0097235 A1          | 4/2011    | Turconi et al.    |         |  |
| 9,383,045 B2          | 7/2016           | Santi et al.         | 2011/0133449 A1          | 6/2011    | Mazzaferro        |         |  |
| 9,598,746 B2          | 3/2017           | Anelli et al.        | 2011/0233925 A1          | 9/2011    | Pina              |         |  |
| 9,708,681 B2          | 7/2017           | Eguchi et al.        | 2011/0247733 A1          | 10/2011   | Arai et al.       |         |  |
| 9,745,640 B2          | 8/2017           | Valdez et al.        | 2011/0259482 A1          | 10/2011   | Peters            |         |  |
| 9,803,256 B2          | 10/2017          | Valdez et al.        | 2011/0284137 A1          | 11/2011   | Kami et al.       |         |  |
| 10,378,074 B2         | 8/2019           | Valdez et al.        | 2012/0018056 A1          | 1/2012    | Nakagawa et al.   |         |  |
| 10,378,075 B2         | 8/2019           | Valdez et al.        | 2012/0186686 A1          | 7/2012    | Valdez            |         |  |
| 10,480,054 B2         | 11/2019          | Valdez et al.        | 2012/0199255 A1          | 8/2012    | Anelli            |         |  |
| 2001/0035235 A1       | 11/2001          | Kawano               | 2012/0267014 A1          | 10/2012   | Hitoshio et al.   |         |  |
| 2002/0011284 A1       | 1/2002           | Von Hagen et al.     | 2013/0000790 A1          | 1/2013    | Arai et al.       |         |  |
| 2002/0153671 A1       | 10/2002          | Raymond et al.       | 2013/0004787 A1          | 1/2013    | Ishiyama et al.   |         |  |
| 2002/0158469 A1       | 10/2002          | Mannella et al.      | 2013/0199674 A1          | 8/2013    | Altschuler et al. |         |  |
| 2003/0019549 A1       | 1/2003           | Turconi et al.       | 2013/0264123 A1          | 10/2013   | Altschuler et al. |         |  |
| 2003/0111146 A1       | 6/2003           | Kusinski et al.      | 2014/0021244 A1          | 1/2014    | DuBois            |         |  |
| 2003/0116238 A1       | 6/2003           | Fujita               | 2014/0027497 A1          | 1/2014    | Rowland et al.    |         |  |
| 2003/0155052 A1       | 8/2003           | Kondo et al.         | 2014/0057121 A1          | 2/2014    | Altschuler et al. |         |  |
| 2003/0165098 A1       | 9/2003           | Ohara et al.         | 2014/0137992 A1          | 5/2014    | Ishiguro et al.   |         |  |
| 2003/0168859 A1       | 9/2003           | Watts                | 2014/0251512 A1          | 9/2014    | Gomez             |         |  |
| 2004/0118490 A1       | 6/2004           | Klueh et al.         | 2014/0272448 A1          | 9/2014    | Valdez et al.     |         |  |
| 2004/0118569 A1       | 6/2004           | Brill et al.         | 2014/0299235 A1          | 10/2014   | Anelli            |         |  |
| 2004/0131876 A1       | 7/2004           | Ohgami et al.        | 2014/0299236 A1          | 10/2014   | Anelli            |         |  |
| 2004/0139780 A1       | 7/2004           | Cai et al.           | 2015/0368986 A1          | 12/2015   | Narikawa          |         |  |
| 2004/0187971 A1       | 9/2004           | Omura                | 2016/0024625 A1          | 1/2016    | Valdez            |         |  |
| 2004/0195835 A1       | 10/2004          | Noel et al.          | 2016/0102856 A1          | 4/2016    | Minami            |         |  |
| 2004/0262919 A1       | 12/2004          | Dutilleul et al.     | 2016/0281188 A1          | 9/2016    | Valdez et al.     |         |  |
| 2005/0012278 A1       | 1/2005           | Delange              | 2016/0305192 A1          | 10/2016   | Buhler            |         |  |
| 2005/0076975 A1       | 4/2005           | Lopez et al.         | 2018/0044747 A1          | 2/2018    | Valdez et al.     |         |  |
| 2005/0087269 A1       | 4/2005           | Merwin               | 2018/0051353 A1          | 2/2018    | Valdez et al.     |         |  |
| 2005/0093250 A1       | 5/2005           | Santi et al.         | FOREIGN PATENT DOCUMENTS |           |                   |         |  |
| 2005/0166986 A1       | 8/2005           | Dell'erba et al.     | CA                       | 2319926   | 7/2008            |         |  |
| 2006/0006600 A1       | 1/2006           | Roussie              | CA                       | 2685001   | 11/2008           |         |  |
| 2006/0124211 A1       | 6/2006           | Takano et al.        | CN                       | 1401809   | 3/2003            |         |  |
| 2006/0137781 A1       | 6/2006           | Kusinski et al.      | CN                       | 1487112   | 4/2004            |         |  |
| 2006/0157539 A1*      | 7/2006           | DuBois .....         | B21C 37/0811             | CN        | 1292429           | 12/2006 |  |
|                       |                  |                      | 228/144                  | CN        | 101480671         | 7/2009  |  |
|                       |                  |                      |                          | CN        | 101542002         | 9/2009  |  |
|                       |                  |                      |                          | CN        | 101613829         | 12/2009 |  |
| 2006/0169368 A1       | 8/2006           | Lopez et al.         | CN                       | 101413089 | 11/2010           |         |  |
| 2006/0231168 A1       | 10/2006          | Nakamura et al.      | CN                       | 101898295 | 12/2010           |         |  |
| 2006/0231186 A1       | 10/2006          | Minami et al.        | DE                       | 3310226   | 10/1984           |         |  |
| 2006/0243355 A1       | 11/2006          | Haiderer et al.      | DE                       | 4446806   | 5/1996            |         |  |
| 2006/0273586 A1       | 12/2006          | Reynolds, Jr. et al. | EA                       | 010037    | 6/2008            |         |  |
| 2007/0039147 A1       | 2/2007           | Roussie              | EA                       | 012256    | 8/2009            |         |  |
| 2007/0039149 A1       | 2/2007           | Roussie              | EP                       | 0032265   | 7/1981            |         |  |
| 2007/0088913 A1       | 4/2007           | Tivelli              | EP                       | 0092815   | 11/1983           |         |  |
| 2007/0137736 A1       | 6/2007           | Omura et al.         | EP                       | 0104720   | 4/1984            |         |  |
| 2007/0216126 A1       | 9/2007           | Lopez et al.         | EP                       | 0159385   | 10/1985           |         |  |
| 2007/0246219 A1       | 10/2007          | Manella et al.       | EP                       | 0309179   | 3/1989            |         |  |
| 2008/0047635 A1       | 2/2008           | Kanda et al.         | EP                       | 0340385   | 11/1989           |         |  |
| 2008/0115863 A1       | 5/2008           | McCrink et al.       | EP                       | 0329990   | 11/1992           |         |  |
| 2008/0129044 A1       | 6/2008           | Carcagno et al.      | EP                       | 0658632   | 6/1995            |         |  |
| 2008/0219878 A1       | 9/2008           | Kanda et al.         | EP                       | 0753595   | 1/1997            |         |  |
| 2008/0226396 A1       | 9/2008           | Garcia et al.        | EP                       | 0788850   | 8/1997            |         |  |
| 2008/0226491 A1       | 9/2008           | Satou et al.         | EP                       | 0828007   | 3/1998            |         |  |
| 2008/0257459 A1       | 10/2008          | Arai et al.          | EP                       | 0989196   | 3/2000            |         |  |
| 2008/0264129 A1       | 10/2008          | Cheppe et al.        | EP                       | 1008660   | 6/2000            |         |  |
| 2008/0286504 A1       | 11/2008          | Asahi et al.         | EP                       | 1027944   | 8/2000            |         |  |
| 2008/0303274 A1       | 12/2008          | Mazzaferro et al.    | EP                       | 1065423   | 1/2001            |         |  |

| (56) | References Cited         | JP | 11 140580       | 5/1999  |
|------|--------------------------|----|-----------------|---------|
|      | FOREIGN PATENT DOCUMENTS | JP | 11 229079       | 8/1999  |
| EP   | 0828007 11/2001          | JP | 2000-063940     | 2/2000  |
| EP   | 1269059 1/2003           | JP | 2000-178645     | 6/2000  |
| EP   | 1277848 1/2003           | JP | 2000-248337     | 9/2000  |
| EP   | 1288316 3/2003           | JP | 2000-313919     | 11/2000 |
| EP   | 1296088 3/2003           | JP | 2001-131698     | 5/2001  |
| EP   | 1362977 11/2003          | JP | 2001-164338     | 6/2001  |
| EP   | 1413639 4/2004           | JP | 2001-172739     | 6/2001  |
| EP   | 1482268 9/2004           | JP | 2001220653 A *  | 8/2001  |
| EP   | 1705415 9/2006           | JP | 2001-271134     | 10/2001 |
| EP   | 1717324 11/2006          | JP | 2002-096105     | 4/2002  |
| EP   | 1726861 11/2006          | JP | 2002-130554     | 5/2002  |
| EP   | 1876254 1/2008           | JP | 2002-0411009    | 1/2004  |
| EP   | 1914324 4/2008           | JP | 60 174822       | 9/2005  |
| EP   | 2000629 12/2008          | KR | 0245031         | 3/2000  |
| EP   | 1554518 1/2009           | KZ | 1418 B          | 12/1994 |
| EP   | 2028284 2/2009           | KZ | 2506 B          | 9/1995  |
| EP   | 2133442 12/2009          | KZ | 2673 B          | 12/1995 |
| EP   | 2447386 2/2010           | UA | 51138 A         | 11/2002 |
| EP   | 2216576 8/2010           | WO | WO 1984/002947  | 8/1984  |
| EP   | 2239343 10/2010          | WO | WO 1994/29627   | 12/1994 |
| EP   | 2729590 1/2013           | WO | WO 1996/22396   | 7/1996  |
| FR   | 1149513 12/1957          | WO | WO 2000/06931   | 2/2000  |
| FR   | 1489013 7/1967           | WO | WO 2000/70107   | 11/2000 |
| FR   | 2 704 042 A 10/1994      | WO | WO 2001/075345  | 10/2001 |
| FR   | 2 848 282 A1 6/2004      | WO | WO 2001/88210   | 11/2001 |
| FR   | 2855587 12/2004          | WO | WO 2002/29290   | 4/2002  |
| GB   | 498472 1/1939            | WO | WO 2002/035128  | 5/2002  |
| GB   | 1 398 214 6/1973         | WO | WO 2002/068854  | 9/2002  |
| GB   | 1 428 433 3/1976         | WO | WO 2002/086369  | 10/2002 |
| GB   | 2 104 919 A 3/1983       | WO | WO 2002/093045  | 11/2002 |
| GB   | 2 234 308 1/1991         | WO | WO 2003/033856  | 4/2003  |
| GB   | 2 276 647 10/1994        | WO | WO 2003/048623  | 6/2003  |
| GB   | 2 388169 11/2003         | WO | WO 2003/087646  | 10/2003 |
| JP   | S522825 1/1977           | WO | WO 2004/023020  | 3/2004  |
| JP   | 58-187684 12/1983        | WO | WO 2004/031420  | 4/2004  |
| JP   | 60-086209 5/1985         | WO | WO 2004/033951  | 4/2004  |
| JP   | S60 11 6796 6/1985       | WO | WO 2004/053376  | 6/2004  |
| JP   | 60-215719 10/1985        | WO | WO 2004/097059  | 11/2004 |
| JP   | 36025719 10/1985         | WO | WO 2004/109173  | 12/2004 |
| JP   | S60215719 10/1985        | WO | WO 2006/003775  | 6/2005  |
| JP   | S60261888 12/1985        | WO | WO 2005/080621  | 9/2005  |
| JP   | S61-103061 5/1986        | WO | WO 2006/009142  | 1/2006  |
| JP   | 61 270355 11/1986        | WO | WO 2006/087361  | 4/2006  |
| JP   | 63 004046 1/1988         | WO | WO2006078768    | 7/2006  |
| JP   | 63 004047 1/1988         | WO | WO2006086143    | 8/2006  |
| JP   | 63-230847 A2 9/1988      | WO | WO 2007/002576  | 1/2007  |
| JP   | 63230851 9/1988          | WO | WO 2007/017082  | 2/2007  |
| JP   | 01-242761 9/1989         | WO | WO 2007/017161  | 2/2007  |
| JP   | 01 259124 10/1989        | WO | WO 2007/023806  | 3/2007  |
| JP   | 01 259125 10/1989        | WO | WO 2007/028443  | 3/2007  |
| JP   | 01 283322 11/1989        | WO | WO 2007/034063  | 3/2007  |
| JP   | 05-098350 12/1990        | WO | WO 2007/063079  | 6/2007  |
| JP   | 403006329 1/1991         | WO | WO 2008/003000  | 1/2008  |
| JP   | 04 021718 1/1992         | WO | WO 2008/007737  | 1/2008  |
| JP   | 04 107214 4/1992         | WO | WO 2008/090411  | 7/2008  |
| JP   | 04 231414 8/1992         | WO | WO 2008/110494  | 9/2008  |
| JP   | H0574928 10/1993         | WO | WO 2008/127084  | 10/2008 |
| JP   | 05 287381 11/1993        | WO | WO 2009/000851  | 12/2008 |
| JP   | H06-042645 2/1994        | WO | WO 2009/000766  | 1/2009  |
| JP   | 06-093339 4/1994         | WO | WO 2009/010507  | 1/2009  |
| JP   | 06 172859 6/1994         | WO | WO 2009/027308  | 3/2009  |
| JP   | 06-220536 8/1994         | WO | WO 2009/027309  | 3/2009  |
| JP   | 07-003330 1/1995         | WO | WO 2009/044297  | 4/2009  |
| JP   | 07 041856 2/1995         | WO | WO 2009/065432  | 5/2009  |
| JP   | 07-139666 5/1995         | WO | WO 2009/106623  | 9/2009  |
| JP   | 07 197125 8/1995         | WO | WO 2010/061882  | 6/2010  |
| JP   | 08 311551 11/1996        | WO | WO 2010/122431  | 10/2010 |
| JP   | 09 067624 3/1997         | WO | WO 2011 /152240 | 12/2011 |
| JP   | H09217120 8/1997         | WO | WO2013007729    | 1/2013  |
| JP   | 09-235617 9/1997         |    |                 |         |
| JP   | 2704042 10/1997          |    |                 |         |
| JP   | 10 140250 5/1998         |    |                 |         |
| JP   | 10 176239 6/1998         |    |                 |         |
| JP   | 10 280037 10/1998        |    |                 |         |
| JP   | 11 050148 2/1999         |    |                 |         |

## OTHER PUBLICATIONS

(56)

**References Cited****OTHER PUBLICATIONS**

in Houston on or about Mar. 28-31, 1994, document bears the date of Mar. 1, 1994, 20 pages (1-20), of the 60 page composite document submitted herewith as Desig. ID 48.

[No Author Listed], "Southwestern Pipe, Inc.—Cymax Coiled Tubing," Unknown if this document was publicly disclosed, Date of publication unknown, but presumably prior to the earliest claimed priority date for the pending application, 1 page (p. 22) of the 60 page composite document submitted herewith as Desig. ID 48.

[No Author Listed], "CYMAX Division—Coiled Tubing Reel Sizes," Unknown if this document was publicly disclosed, Date of publication unknown, but presumably prior to the earliest claimed priority date for the pending application, 1 page (p. 24) of the 60 page composite document submitted herewith as Desig. ID 48.

[No Author Listed], "Coiled Tubing String Design," Unknown if this document was publicly disclosed, Date of publication unknown, but presumably prior to the earliest claimed priority date for the pending application, 2 pages (25- 26) of the 60 page composite document submitted herewith as Desig. ID 48.

"Southwestern Pipe Inc., Specification for Cymax 80 High Strength Low Alloy Steel Coiled Tubing for Sour Environment Service," Date of publication unknown, but presumably prior to the earliest claimed priority date for the pending application; document bears the date Sep. 1, 1993, 2 pages (28-29) of the 60 page composite document submitted herewith as Desig. ID 48.

"Southwestern Pipe Inc., Specification for Cymax 100 High Strength Low Alloy Steel Coiled Tubing for Sour Environment Service," Date of publication unknown, but presumably prior to the earliest claimed priority date for the pending application; document bears the date Sep. 1, 1993, 2 pages (30-31) of the 60 page composite document submitted herewith as Desig. ID 48.

[No Author Listed], "The Development and Testing of CYMAX 100 Coiled Tubing," Date of publication unknown, but presumably prior to the earliest claimed priority date for the pending application; document bears the date Jan. 1992 and is cited in the bibliography of the Full Body Quenched and Tempered Coiled Tubing dated Mar. 1, 1994, 15 pages (33-47) of the 60 page composite document submitted herewith as Desig. ID 48.

[No Author Listed], "Orbital TIG Welding Cymax Coiled Tubing," Unknown if this document was publicly disclosed, Date of publication unknown, but presumably prior to the earliest claimed priority date for the pending application; document bears the date Nov. 1992, 13 pages (48-60) of the 60 page composite document submitted herewith as Desig. ID 48.

Divider Pages labeled "Southwestern Pipe Inc.;" "CYMAX Division;" "Coiled Tubing Specifications;" "Technical Data—Introduction;" "Product Data—Specifications—Technical Papers" Date of publication unknown, but presumably prior to the earliest claimed priority date for the pending application; 4 pages (21, 23, 27, and 32) of the 60 page composite document submitted herewith as Desig. ID 48.

"Untitled Composite of Multiple Documents", Cymax Division, Southwestern Pipe, Inc.; Date of publication unknown, but presumably prior to the earliest claimed priority date for the pending application, document bears the date of Mar. 1, 1994, 60 pages; document is a composite of the documents submitted herewith as Desig. ID Nos. 39-47.

Chitwood, G. B., et al.: "High-Strength Coiled Tubing Expands Service Capabilities", as presented at the 24th Annual OTC in Houston, Texas, May 4-7, 1992, 15 pages.

Chinese Office Action for Application No. 201210020833.5 with English Translation dated on May 5, 2015.

European Extended Search Report re EPO Application No. 12152516.6, dated Jun. 25, 2012.

European Search Report and Opinion, re EPO Application No. EP 14159174.3, dated Jul. 3, 2014.

Fazsold et al., "Full-Scale Fatigue Testing With 130K Yield Tubing," Paper SPE-153945, Presented at SPE/ICoTA Coiled Tubing & Well Intervention Conference and Exhibition Jan. 2012, Society of Petroleum Engineers, 6 pages.

First Chinese Office Action for Application No. 201210020833.5 with English Translation dated on Aug. 4, 2014.

Hollomon, J.H., et al., Time-tempered Relations in Tempering Steel. New York Meeting, 1945, pp. 223-249.

International Standard Publication. Petroleum and natural gas industries—Materials for use in H2S-containing environments in oil and gas production. ANSI/NACE ISO, 2009, 145 pages.

Pollack, Herman, W., Materials Science and Metallurgy, Fourth Edition, pp. 96 and 97, 1988, 2 pages.

Savatori et. al. European Commision Report, EUR 2006, EUR2207, STN Abstract, 3 pages.

Tenaris brochure. Coiled Tubes HS8OCRA, 2 pages, 2008.

Tenaris brochure. Coiled Tubes Suggested Field Welding Procedure (GTAW) for Coiled Tubing Grads HS70, HS80, HS90, HS110, 2007, 3 pages.

Tenaris brochure. Coiled Tubing for Downhole Applications, 2007, 10 pages.

Docket sheet from *Global Tubing, LLC vs. Tenaris Coiled Tubes, LLC et al.*, case No. 4:17-cv-03299 in the United States District Court for the Southern District of Texas, Houston Division, 31 pages.

United States District Court for the Southern District of Texas, Houston Division, Global's Final Invalidity Contentions, Civil Action No. 4:17-cv-03299, dated Apr. 12, 2021, 59 pages.

Exhibit A-1 Identification of Asserted Claims and Limitations Therein, U.S. Pat. No. 9,803,256, served by Global Tubing, LLC on Apr. 12, 2021 in *Global Tubing, LLC vs. Tenaris Coiled Tubes, LLC et al.*, case No. 4:17-cv-03299 in the United States District Court for the Southern District of Texas, Houston Division, 19 pages. Exhibit A-2 U.S. Pat. No. 9,803,256, served by Global Tubing, LLC on Apr. 12, 2021 in *Global Tubing, LLC vs. Tenaris Coiled Tubes, LLC et al.*, case No. 4:17-cv-03299 in the United States District Court for the Southern District of Texas, Houston Division, 19 pages.

Exhibit A-3 Altschuler 715, served by Global Tubing, LLC on Apr. 12, 2021 (and referring to a document beginning with p. GT0011425) in *Global Tubing, LLC vs. Tenaris Coiled Tubes, LLC et al.*, case No. 4:17-cv-03299 in the United States District Court for the Southern District of Texas, Houston Division, 19 pages.

Exhibit A-3 Altschuler 856, served by Global Tubing, LLC on Apr. 12, 2021 (and referring to a document beginning with p. GT0011442) in *Global Tubing, LLC vs. Tenaris Coiled Tubes, LLC et al.*, case No. 4:17-cv-03299 in the United States District Court for the Southern District of Texas, Houston Division, 17 pages.

Exhibit A-3 API Specification, American Petroleum Institute, Specification for Coiled Tubing, API Specification 5ST, served by Global Tubing, LLC on Apr. 12, 2021 (and referring to a document beginning with p. GT0224055) in *Global Tubing, LLC vs. Tenaris Coiled Tubes, LLC et al.*, case No. 4:17-cv-03299 in the United States District Court for the Southern District of Texas, Houston Division, 13 pages.

Exhibit A-3 Asano (Supplemental), served by Global Tubing, LLC on Apr. 12, 2021 (and referring to documents beginning with p. GT0011542 and GT0011547) in *Global Tubing, LLC vs. Tenaris Coiled Tubes, LLC et al.*, case No. 4:17-cv-03299 in the United States District Court for the Southern District of Texas, Houston Division, 18 pages.

Exhibit A-3 Chitwood, High Strength Coiled Tubing Expands Service Capabilities, served by Global Tubing on Apr. 12, 2021 (and referring to a document beginning with p. GT0023898 and ending with p. GT0023913) in *Global Tubing, LLC vs. Tenaris Coiled Tubes, LLC et al.*, case No. 4:17-cv-03299 in the United States District Court for the Southern District of Texas, Houston Division, 28 pages.

Exhibit A-3 Crowther, served by Global Tubing, LLC on Apr. 12, 2021 (and referring to a document beginning with p. GT0012789) in *Global Tubing, LLC vs. Tenaris Coiled Tubes, LLC et al.*, case No. 4:17-cv-03299 in the United States District Court for the Southern District of Texas, Houston Division, 23 pages.

Exhibit A-3 CT Manual (Supplemental), Coiled Tubing Manual, served by Global Tubing, LLC on Apr. 12, 2021 (and referring to a document beginning with p. GT0011855) in *Global Tubing, LLC vs.*

(56)

**References Cited****OTHER PUBLICATIONS**

*Tenaris Coiled Tubes, LLC et al.*, case No. 4:17-cv-03299 in the United States District Court for the Southern District of Texas, Houston Division, 15 pages.

Exhibit A-3 CYMAX 100, served by Global Tubing, LLC on Apr. 12, 2021 in *Global Tubing, LLC vs. Tenaris Coiled Tubes, LLC et al.*, case No. 4:17-cv-03299 in the United States District Court for the Southern District of Texas, Houston Division, 22 pages.

Exhibit A-3 CYMAX Brochure, served by Global Tubing, LLC on Apr. 12, 2021 (and referring to a document labeled with pp. TCT0009950-89) in *Global Tubing, LLC vs. Tenaris Coiled Tubes, LLC et al.*, case No. 4:17-cv-03299 in the United States District Court for the Southern District of Texas, Houston Division, 21 pages.

Exhibit A-3 Eguchi 681, served by Global Tubing, LLC on Apr. 12, 2021 (and referring to a document beginning with p. GT0012866 and ending with p. GT0012878) in *Global Tubing, LLC vs. Tenaris Coiled Tubes, LLC et al.*, case No. 4:17-cv-03299 in the United States District Court for the Southern District of Texas, Houston Division, 26 pages.

Exhibit A-3 Eguchi 2012, served by Global Tubing, LLC on Apr. 12, 2021 (and referring to a document beginning with p. GT0012879) in *Global Tubing, LLC vs. Tenaris Coiled Tubes, LLC et al.*, case No. 4:17-cv-03299 in the United States District Court for the Southern District of Texas, Houston Division, 24 pages.

Exhibit A-3 Feng, served by Global Tubing, LLC on Apr. 12, 2021 (and referring to a document beginning with p. GT0283198) in *Global Tubing, LLC vs. Tenaris Coiled Tubes, LLC et al.*, case No. 4:17-cv-03299 in the United States District Court for the Southern District of Texas, Houston Division, 15 pages.

Exhibit A-3 Fujishiro, served by Global Tubing, LLC on Apr. 12, 2021 (and referring to a document beginning with p. GT0025074 and ending with p. GT0025083) in *Global Tubing, LLC vs. Tenaris Coiled Tubes, LLC et al.*, case No. 4:17-cv-03299 in the United States District Court for the Southern District of Texas, Houston Division, 21 pages.

Exhibit A-3 Kushida, served by Global Tubing, LLC on Apr. 12, 2021 (and referring to a document beginning with p. GT0012967) in *Global Tubing, LLC vs. Tenaris Coiled Tubes, LLC et al.*, case No. 4:17-cv-03299 in the United States District Court for the Southern District of Texas, Houston Division, 22 pages.

Exhibit A-3 O'Hara, served by Global Tubing, LLC on Apr. 12, 2021 (and referring to a document beginning with p. GT0025287) in *Global Tubing, LLC vs. Tenaris Coiled Tubes, LLC et al.*, case No. 4:17-cv-03299 in the United States District Court for the Southern District of Texas, Houston Division, 14 pages.

Exhibit A-3 Peters, served by Global Tubing, LLC on Apr. 12, 2021 (and referring to a document beginning with p. GT0013047) in *Global Tubing, LLC vs. Tenaris Coiled Tubes, LLC et al.*, case No. 4:17-cv-03299 in the United States District Court for the Southern District of Texas, Houston Division, 20 pages.

Exhibit A-3 Satou, served by Global Tubing, LLC on Apr. 12, 2021 (and referring to a document beginning with p. GT0025646) in *Global Tubing, LLC vs. Tenaris Coiled Tubes, LLC et al.*, case No. 4:17-cv-03299 in the United States District Court for the Southern District of Texas, Houston Division, 17 pages.

Exhibit A-3 SeaCAT 100, served by Global Tubing, LLC on Apr. 12, 2021 (and referring to documents beginning with p. TCT0374366, GT0210506, TCT0373809, TCT0372631, GT0011295, TCT0372486, TCT0375105, TCT03727329-TCT0374535) in *Global Tubing, LLC vs. Tenaris Coiled Tubes, LLC et al.*, case No. 4:17-cv-03299 in the United States District Court for the Southern District of Texas, Houston Division, 16 pages.

Exhibit A-3 SeaCAT Specification, served by Global Tubing, LLC on Apr. 12, 2021 (and referring to a document beginning with p. GT0210506) in *Global Tubing, LLC vs. Tenaris Coiled Tubes, LLC et al.*, case No. 4:17-cv-03299 in the United States District Court for the Southern District of Texas, Houston Division, 12 pages.

Exhibit A-3 Takeshi, served by Global Tubing, LLC on Apr. 12, 2021 (and referring to a document beginning with p. GT0025731)

in *Global Tubing, LLC vs. Tenaris Coiled Tubes, LLC et al.*, case No. 4:17-cv-03299 in the United States District Court for the Southern District of Texas, Houston Division, 17 pages.

Exhibit A-3 Thompson, served by Global Tubing, LLC on Apr. 12, 2021 (and referring to a document labeled with pp. TCT0009930-49) in *Global Tubing, LLC vs. Tenaris Coiled Tubes, LLC et al.*, case No. 4:17-cv-03299 in the United States District Court for the Southern District of Texas, Houston Division, 21 pages.

Exhibit A-3 Turconi, served by Global Tubing, LLC on Apr. 12, 2021 (and referring to a document beginning with p. GT0011237) in *Global Tubing, LLC vs. Tenaris Coiled Tubes, LLC et al.*, case No. 4:17-cv-03299 in the United States District Court for the Southern District of Texas, Houston Division, 22 pages.

Exhibit A-3 Turconi 2001, served by Global Tubing, LLC on Apr. 12, 2021 (and referring to a document beginning with p. GT0025769) in *Global Tubing, LLC vs. Tenaris Coiled Tubes, LLC et al.*, case No. 4:17-cv-03299 in the United States District Court for the Southern District of Texas, Houston Division, 19 pages.

Exhibit A-3 Valdez 2010, served by Global Tubing, LLC on Apr. 12, 2021 (and referring to a document beginning with p. GT0011261) in *Global Tubing, LLC vs. Tenaris Coiled Tubes, LLC et al.*, case No. 4:17-cv-03299 in the United States District Court for the Southern District of Texas, Houston Division, 16 pages.

Exhibit A-3 Williams, served by Global Tubing, LLC on Apr. 12, 2021 (and referring to a document beginning with p. GT0011295) in *Global Tubing, LLC vs. Tenaris Coiled Tubes, LLC et al.*, case No. 4:17-cv-03299 in the United States District Court for the Southern District of Texas, Houston Division, 13 pages.

Exhibit A-3 Zernick, served by Global Tubing, LLC on Apr. 12, 2021 (and referring to a document beginning with p. GT0011300) in *Global Tubing, LLC vs. Tenaris Coiled Tubes, LLC et al.*, case No. 4:17-cv-03299 in the United States District Court for the Southern District of Texas, Houston Division, 18 pages.

Exhibit B-1, Identification of Asserted Claims and Limitations Therein, U.S. Pat. No. 10,378,074, served by Global Tubing, LLC on Apr. 12, 2021 in *Global Tubing, LLC vs. Tenaris Coiled Tubes, LLC et al.*, case No. 4:17-cv-03299 in the United States District Court for the Southern District of Texas, Houston Division, 4 pages.

Exhibit B-2, U.S. Pat. No. 10,378,074, 28 pages with Exhibit B-3 Attachments totaling 233 pages, served by Global Tubing, LLC on Apr. 12, 2021 in *Global Tubing, LLC vs. Tenaris Coiled Tubes, LLC et al.*, case No. 4:17-cv-03299 in the United States District Court for the Southern District of Texas, Houston Division.

Exhibit B-3 Altschuler 715, served by Global Tubing, LLC on Apr. 12, 2021 (and referring to a document beginning with p. GT0011425) in *Global Tubing, LLC vs. Tenaris Coiled Tubes, LLC et al.*, case No. 4:17-cv-03299 in the United States District Court for the Southern District of Texas, Houston Division, 9 pages.

Exhibit B-3 Altschuler 856, served by Global Tubing, LLC on Apr. 12, 2021 (and referring to a document beginning with p. GT0011442) in *Global Tubing, LLC vs. Tenaris Coiled Tubes, LLC et al.*, case No. 4:17-cv-03299 in the United States District Court for the Southern District of Texas, Houston Division, 8 pages.

Exhibit B-3 API Specification, American Petroleum Institute, Specification for Coiled Tubing, API Specification 5ST, served by Global Tubing, LLC on Apr. 12, 2021 (and referring to a document beginning with p. GT0224055) in *Global Tubing, LLC vs. Tenaris Coiled Tubes, LLC et al.*, case No. 4:17-cv-03299 in the United States District Court for the Southern District of Texas, Houston Division, 7 pages.

Exhibit B-3 Asano (Supplemental), served by Global Tubing, LLC on Apr. 12, 2021 (and referring to documents beginning with p. GT0011542 and GT0011547) in *Global Tubing, LLC vs. Tenaris Coiled Tubes, LLC et al.*, case No. 4:17-cv-03299 in the United States District Court for the Southern District of Texas, Houston Division, 7 pages.

Exhibit B-3 Chitwood, High Strength Coiled Tubing Expands Service Capabilities, served by Global Tubing on Apr. 12, 2021 (and referring to a document beginning with p. GT0023898 and ending with p. GT0023913) in *Global Tubing, LLC vs. Tenaris Coiled Tubes, LLC et al.*, case No. 4:17-cv-03299 in the United States District Court for the Southern District of Texas, Houston Division, 7 pages.

(56)

**References Cited****OTHER PUBLICATIONS**

Exhibit B-3 Crowther, served by Global Tubing, LLC on Apr. 12, 2021 (and referring to a document beginning with p. GT0012789) in *Global Tubing, LLC vs. Tenaris Coiled Tubes, LLC et al.*, case No. 4:17-cv-03299 in the United States District Court for the Southern District of Texas, Houston Division, 10 pages.

Exhibit B-3 CT Manual (Supplemental), Coiled Tubing Manual, served by Global Tubing, LLC on Apr. 12, 2021 (and referring to a document beginning with p. GT0011855) in *Global Tubing, LLC vs. Tenaris Coiled Tubes, LLC et al.*, case No. 4:17-cv-03299 in the United States District Court for the Southern District of Texas, Houston Division, 7 pages.

Exhibit B-3 CYMAX 100, served by Global Tubing, LLC on Apr. 12, 2021 in *Global Tubing, LLC vs. Tenaris Coiled Tubes, LLC et al.*, case No. 4:17-cv-03299 in the United States District of Texas, Houston Division, 8 pages.

Exhibit B-3 CYMAX Brochure, served by Global Tubing, LLC on Apr. 12, 2021 (and referring to a document labeled with pp. TCT0009950-89) in *Global Tubing, LLC vs. Tenaris Coiled Tubes, LLC et al.*, case No. 4:17-cv-03299 in the United States District Court for the Southern District of Texas, Houston Division, 7 pages. Exhibit B-3 Eguchi 681, served by Global Tubing, LLC on Apr. 12, 2021 (and referring to a document beginning with p. GT0012866 and ending with p. GT0012878) in *Global Tubing, LLC vs. Tenaris Coiled Tubes, LLC et al.*, case No. 4:17-cv-03299 in the United States District Court for the Southern District of Texas, Houston Division 11 pages.

Exhibit B-3 Eguchi 2012, served by Global Tubing, LLC on Apr. 12, 2021 (and referring to a document beginning with p. GT0012879) in *Global Tubing, LLC vs. Tenaris Coiled Tubes, LLC et al.*, case No. 4:17-cv-03299 in the United States District Court for the Southern District of Texas, Houston Division, 12 pages.

Exhibit B-3 Feng, served in Global Tubing, LLC on Apr. 12, 2021 (and referring to a document beginning with p. GT0283198) in *Global Tubing, LLC vs. Tenaris Coiled Tubes, LLC et al.*, case No. 4:17-cv-03299 in the United States District Court for the Southern District of Texas, Houston Division 10 pages.

Exhibit B-3 Fujishiro, served in Global Tubing, LLC on Apr. 12, 2021 (and referring to a document beginning with p. GT0025074 and ending with p. GT0025083) in *Global Tubing, LLC vs. Tenaris Coiled Tubes, LLC et al.*, case No. 4:17-cv-03299 in the United States District Court for the Southern District of Texas, Houston Division, 10 pages.

Exhibit B-3 Kushida, served in Global Tubing, LLC on Apr. 12, 2021 (and referring to a document beginning with p. GT0012967) in *Global Tubing, LLC vs. Tenaris Coiled Tubes, LLC et al.*, case No. 4:17-cv-03299 in the United States District Court for the Southern District of Texas, Houston Division, 13 pages.

Exhibit B-3 O'Hara, served by Global Tubing, LLC on Apr. 12, 2021 (and referring to a document beginning with p. GT0025287) in *Global Tubing, LLC vs. Tenaris Coiled Tubes, LLC et al.*, case No. 4:17-cv-03299 in the United States District Court for the Southern District of Texas, Houston Division, 6 pages.

Exhibit B-3 Peters, served by Global Tubing, LLC on Apr. 12, 2021 (and referring to a document beginning with p. GT0013047) in *Global Tubing, LLC vs. Tenaris Coiled Tubes, LLC et al.*, case No. 4:17-cv-03299 in the United States District Court for the Southern District of Texas, Houston Division, 19 pages.

Exhibit B-3 Satou, served by Global Tubing, LLC on Apr. 12, 2021 (and referring to a document beginning with p. GT0025646) in *Global Tubing, LLC vs. Tenaris Coiled Tubes, LLC et al.*, case No. 4:17-cv-03299 in the United States District Court for the Southern District of Texas, Houston Division, 9 pages.

Exhibit B-3 SeaCAT 100, served by Global Tubing, LLC on Apr. 12, 2021 (and referring to documents beginning with p. TCT0374366, GT0210506, TCT0373809, TCT0372631, GT0011295, TCT0372486, TCT0375105, TCT0372730, TCT0374535) in *Global Tubing, LLC vs. Tenaris Coiled Tubes, LLC et al.*, case No. 4:17-cv-03299 in the United States District Court for the Southern District of Texas, Houston Division, 8 pages.

Exhibit B-3 SeaCAT Specification, served by Global Tubing, LLC on Apr. 12, 2021 (and referring to a document beginning with p. GT0210506) in *Global Tubing, LLC vs. Tenaris Coiled Tubes, LLC et al.*, case No. 4:17-cv-03299 in the United States District Court for the Southern District of Texas, Houston Division, 7 pages.

Exhibit B-3 Takeshi, served by Global Tubing, LLC on Apr. 12, 2021 (and referring to a document beginning with p. GT0025731) in *Global Tubing, LLC vs. Tenaris Coiled Tubes, LLC et al.*, case No. 4:17-cv-03299 in the United States District Court for the Southern District of Texas, Houston Division, 8 pages.

Exhibit B-3 Thompson, served by Global Tubing, LLC on Apr. 12, 2021 (and referring to a document labeled with pp. TCT0009930-49) in *Global Tubing, LLC vs. Tenaris Coiled Tubes, LLC et al.*, case No. 4:17-cv-03299 in the United States District Court for the Southern District of Texas, Houston Division, 7 pages.

Exhibit B-3 Turconi, served by Global Tubing, LLC on Apr. 12, 2021 (and referring to a document beginning with p. GT0011237) in *Global Tubing, LLC vs. Tenaris Coiled Tubes, LLC et al.*, case No. 4:17-cv-03299 in the United States District Court for the Southern District of Texas, Houston Division, 11 pages.

Exhibit B-3 Turconi 2001, served by Global Tubing, LLC on Apr. 12, 2021 (and referring to a document beginning with p. GT0025769) in *Global Tubing, LLC vs. Tenaris Coiled Tubes, LLC et al.*, case No. 4:17-cv-03299 in the United States District Court for the Southern District of Texas, Houston Division, 11 pages.

Exhibit B-3 Valdez 2010, served by Global Tubing, LLC on Apr. 12, 2021 (and referring to a document beginning with p. GT0011261) in *Global Tubing, LLC vs. Tenaris Coiled Tubes, LLC et al.*, case No. 4:17-cv-03299 in the United States District Court for the Southern District of Texas, Houston Division, 7 pages.

Exhibit B-3 Williams, served by Global Tubing, LLC on Apr. 12, 2021 (and referring to a document beginning with p. GT0011295) in *Global Tubing, LLC vs. Tenaris Coiled Tubes, LLC et al.*, case No. 4:17-cv-03299 in the United States District Court for the Southern District of Texas, Houston Division , 7 pages.

Exhibit B-3 Zernick, served by Global Tubing, LLC on Apr. 12, 2021 (and referring to a document beginning with p. GT0011300) in *Global Tubing, LLC vs. Tenaris Coiled Tubes, LLC et al.*, case No. 4:17-cv-03299 in the United States District Court for the Southern District of Texas, Houston Division , 7 pages.

Exhibit C-1, Identification of Asserted Claims and Limitations Therein, U.S. Pat. No. 10,378,075, served by Global Tubing, LLC on Apr. 12, 2021 in *Global Tubing, LLC vs. Tenaris Coiled Tubes, LLC et al.*, case No. 4:17-cv-03299 in the United States District Court for the Southern District of Texas, Houston Division, 4 pages. Exhibit C-2, U.S. Pat. No. 10,378,075, served by Global Tubing, LLC on Apr. 12, 2021 in *Global Tubing, LLC vs. Tenaris Coiled Tubes, LLC et al.*, case No. 4:17-cv-03299 in the United States District Court for the Southern District of Texas, Houston Division, 6 pages with Exhibit C-3 Attachments totaling 260 pages.

Exhibit C-3 Altschuler 715, served by Global Tubing, LLC on Apr. 12, 2021 (and referring to a document beginning with p. GT0011425) in *Global Tubing, LLC vs. Tenaris Coiled Tubes, LLC et al.*, case No. 4:17-cv-03299 in the United States District Court for the Southern District of Texas, Houston Division, 5 pages.

Exhibit C-3 Altschuler 856, served by Global Tubing, LLC on Apr. 12, 2021 (and referring to a document beginning with p. GT0011442) in *Global Tubing, LLC vs. Tenaris Coiled Tubes, LLC et al.*, case No. 4:17-cv-03299 in the United States District Court for the Southern District of Texas, Houston Division, 5 pages.

Exhibit C-3 API Specification, American Petroleum Institute, Specification for Coiled Tubing, API Specification 5ST, served by Global Tubing, LLC on Apr. 12, 2021 (and referring to a document beginning with No. GT0224055) in *Global Tubing, LLC vs. Tenaris Coiled Tubes, LLC et al.*, case No. 4:17-cv-03299 in the United States District Court for the Southern District of Texas, Houston Division, 5 pages.

Exhibit C-3 Asano (Supplemental), served by Global Tubing, LLC on Apr. 12, 2021 (and referring to documents beginning with p. GT0011542 and GT0011547) in *Global Tubing, LLC vs. Tenaris Coiled Tubes, LLC et al.*, case No. 4:17-cv-03299 in the United States District Court for the Southern District of Texas, Houston Division, 5 pages.

(56)

**References Cited****OTHER PUBLICATIONS**

Exhibit C-3 Chitwood, High Strength Coiled Tubing Expands Service Capabilities, served by Global Tubing, LLC on Apr. 12, 2021 (and referring to a document beginning with p. GT0023898 and ending with p. GT0023913) in *Global Tubing, LLC vs. Tenaris Coiled Tubes, LLC et al.*, case No. 4:17-cv-03299 in the United States District Court for the Southern District of Texas, Houston Division, 5 pages.

Exhibit C-3 Crowther, served by Global Tubing, LLC on Apr. 12, 2021 (and referring to a document beginning with p. GT0012789) in *Global Tubing, LLC, vs. Tenaris Coiled Tubes, LLC et al.*, case No. 4:17-cv-03299 in the United States District Court for the Southern District of Texas, Houston Division, 5 pages.

Exhibit C-3 CT Manual (Supplemental), Coiled Tubing Manual, served by Global Tubing, LLC on Apr. 12, 2021 (and referring to a document beginning with p. GT0011855) in *Global Tubing, LLC vs. Tenaris Coiled Tubes, LLC et al.*, case No. 4:17-cv-03299 in the United States District Court for the Southern District of Texas, Houston Division, 5 pages.

Exhibit C-3 CYMAX 100, served by Global Tubing, LLC on Apr. 12, 2021 in *Global Tubing, LLC vs. Tenaris Coiled Tubes, LLC et al.*, case No. 4:17-cv-03299 in the United States District of Texas, Houston Division, 5 pages.

Exhibit C-3 CYMAX Brochure, served by Global Tubing, LLC on Apr. 12, 2021 (and referring to a document labeled with pp. TCT0009950-89) in *Global Tubing, LLC vs. Tenaris Coiled Tubes, LLC et al.*, case No. 4:17-cv-03299 in the United States District Court for the Southern District of Texas, Houston Division, 5 pages.

Exhibit C-3 Eguchi 681, served by Global Tubing, LLC on Apr. 12, 2021 (and referring to a document beginning with p. GT0012866 and ending with p. GT0012878) in *Global Tubing, LLC vs. Tenaris Coiled Tubes, LLC et al.*, case No. 4:17-cv-03299 in the United States District Court for the Southern District of Texas, Houston Division, 5 pages.

Exhibit C-3 Eguchi 2012, served by Global Tubing, LLC on Apr. 12, 2021 (and referring to a document beginning with p. GT0012879) in *Global Tubing, LLC vs. Tenaris Coiled Tubes, LLC et al.*, case No. 4:17-cv-03299 in the United States District Court for the Southern District of Texas, Houston Division, 5 pages.

Exhibit C-3 Feng, served in Global Tubing, LLC on Apr. 12, 2021 (and referring to a document beginning with p. GT0283198) in *Global Tubing, LLC, vs Tenaris Coiled Tubes, LLC et al.*, case No. 4:17-cv-03299 in the United States District Court for the Southern District of Texas, Houston Division, 5 pages.

Exhibit C-3 Fujishiro, served in Global Tubing, LLC on Apr. 12, 2021 (and referring to a document beginning with p. GT0025074 and ending with p. GT0025083) in *Global Tubing, LLC, vs Tenaris Coiled Tubes, LLC et al.*, case No. 4:17-cv-03299 in the United States District Court for the Southern District of Texas, Houston Division, 5 pages.

Exhibit C-3 Kushida, served in Global Tubing, LLC on Apr. 12, 2021 (and referring to a document beginning with p. GT0012967) in *Global Tubing, LLC vs. Tenaris Coiled Tubes, LLC et al.*, case No. 4:17-cv-03299 in the United States District Court for the Southern District of Texas, Houston Division, 5 pages.

Exhibit C-3 O'Hara, served by Global Tubing, LLC on Apr. 12, 2021 (and referring to a document beginning with p. GT0025287) in *Global Tubing, LLC vs. Tenaris Coiled Tubes, LLC et al.*, case No. 4:17-cv-03299 in the United States District Court for the Southern District of Texas, Houston Division, 5 pages.

Exhibit C-3 Peters, served by Global Tubing, LLC on Apr. 12, 2021 (and referring to a document beginning with p. GT0013047) in *Global Tubing, LLC vs. Tenaris Coiled Tubes, LLC et al.*, case No. 4:17-cv-03299 in the United States District Court for the Southern District of Texas, Houston Division, 5 pages.

Exhibit C-3 Satou, served by Global Tubing, LLC on Apr. 12, 2021 (and referring to a document beginning with p. GT0025646) in *Global Tubing, LLC vs. Tenaris Coiled Tubes, LLC et al.*, case No. 4:17-cv-03299 in the United States District Court for the Southern District of Texas, Houston Division, 5 pages.

Exhibit C-3 SeaCAT 100, served by Global Tubing, LLC on Apr. 12, 2021 (and referring to documents beginning with p. TCT0374366, GT0210506, TCT0373809, TCT0372631, GT0011295, TCT0372486, TCT0375105, TCT0372730, TCT0374535) in *Global Tubing, LLC vs. Tenaris Coiled Tubes, LLC et al.*, case No. 4:17-cv-03299 in the United States District Court for the Southern District of Texas, Houston Division, 5 pages.

Exhibit C-3 SeaCAT Specification, served by Global Tubing, LLC on Apr. 12, 2021 (and referring to a document beginning with p. GT0210506) in *Global Tubing, LLC vs. Tenaris Coiled Tubes, LLC et al.*, case No. 4:17-cv-03299 in the United States District Court for the Southern District of Texas, Houston Division, 5 pages.

Exhibit C-3 Takeshi, served by Global Tubing, LLC on Apr. 12, 2021 (and referring to a document beginning with p. GT0025731) in *Global Tubing, LLC vs. Tenaris Coiled Tubes, LLC et al.*, case No. 4:17-cv-03299 in the United States District Court for the Southern District of Texas, Houston Division, 5 pages.

Exhibit C-3 Thompson, served by Global Tubing, LLC on Apr. 12, 2021 (and referring to a document labeled with pp. TCT0009930-49) in *Global Tubing, LLC vs. Tenaris Coiled Tubes, LLC et al.*, case No. 4:17-cv-03299 in the United States District Court for the Southern District of Texas, Houston Division, 5 pages.

Exhibit C-3 Turconi, served by Global Tubing, LLC on Apr. 12, 2021 (and referring to a document beginning with p. GT0011237) in *Global Tubing, LLC vs. Tenaris Coiled Tubes, LLC et al.*, case No. 4:17-cv-03299 in the United States District Court for the Southern District of Texas, Houston Division, 5 pages.

Exhibit C-3 Turconi 2001, served by Global Tubing, LLC on Apr. 12, 2021 (and referring to a document beginning with p. GT0025769) in *Global Tubing, LLC vs. Tenaris Coiled Tubes, LLC et al.*, case No. 4:17-cv-03299 in the United States District Court for the Southern District of Texas, Houston Division, 5 pages.

Exhibit C-3 Valdez 2010, served by Global Tubing, LLC on Apr. 12, 2021 (and referring to a document beginning with p. GT0011261) in *Global Tubing, LLC vs. Tenaris Coiled Tubes, LLC et al.*, case No. 4:17-cv-03299 in the United States District Court for the Southern District of Texas, Houston Division, 5 pages.

Exhibit C-3 Williams, served by Global Tubing, LLC on Apr. 12, 2021 (and referring to a document beginning with p. GT0011295) in *Global Tubing, LLC vs. Tenaris Coiled Tubes, LLC et al.*, case No. 4:17-cv-03299 in the United States District Court for the Southern District of Texas, Houston Division, 5 pages.

Exhibit C-3 Zernick, served by Global Tubing, LLC on Apr. 12, 2021 (and referring to a document beginning with p. GT0011300) in *Global Tubing, LLC vs. Tenaris Coiled Tubes, LLC et al.*, case No. 4:17-cv-03299 in the United States District Court for the Southern District of Texas, Houston Division, 5 pages.

U.S. Pat. No. 5,662,145, dated Sep. 2, 1997, served by Global Tubing, LLC on Apr. 12, 2021 as Nos. GT0011220-GT0011231 in *Global Tubing, LLC vs. Tenaris Coiled Tubes, LLC et al.*, case No. 4:17-cv-03299 in the United States District Court for the Southern District of Texas, Houston Division, 12 pages.

Timkin "Practical Data for Metallurgists", published 1993, served by Global Tubing, LLC on Apr. 12, 2021 as Nos. GT0011232-GT0011236 in *Global Tubing, LLC vs. Tenaris Coiled Tubes, LLC et al.*, case No. 4:17-cv-03299 in the United States District Court for the Southern District of Texas, Houston Division, 5 pages.

U.S. Pat. No. 7,862,667, dated Jan. 4, 2011, served by Global Tubing, LLC on Apr. 12, 2021 as Nos. GT0011237-GT0011252 in *Global Tubing, LLC vs. Tenaris Coiled Tubes, LLC et al.*, case No. 4:17-cv-03299 in the United States District Court for the Southern District of Texas, Houston Division, 16 pages.

Urayama et al., "Research and Development of Advanced Coiled-Tubing Construction and Performance", published Jun. 1, 2001, served by Global Tubing, LLC on Apr. 12, 2021 as Nos. GT0011253-GT0011260 in *Global Tubing, LLC vs. Tenaris Coiled Tubes, LLC et al.*, case No. 4:17-cv-03299 in the United States District Court for the Southern District of Texas, Houston Division, 8 pages.

United States Publication No. 2010/0136363 A1, Jun. 3, 2010, served by Global Tubing, LLC on Apr. 12, 2021 as Nos. GT0011261-GT0011279 in *Global Tubing, LLC vs. Tenaris Coiled Tubes, LLC et al.*, case No. 4:17-cv-03299 in the United States District Court for the Southern District of Texas, Houston Division, 19 pages.

(56)

## References Cited

## OTHER PUBLICATIONS

- Williams, et al., "Mensa Project: Hydraulic Umbilicals", OTC 8629, Offshore Technology Conference, 1998, served by Global Tubing, LLC on Apr. 12, 2021 as Nos. GT0011295-GT0011299 in *Global Tubing, LLC vs. Tenaris Coiled Tubes, LLC et al.*, case No. 4:17-cv-03299 in the United States District Court for the Southern District of Texas, Houston Division, 5 pages.
- Zernick, Bill, "The Development and testing of CYMAX 100 Coiled Tubing", from "Benefits of full body quench and tempered coiled tubing", First Annual Conference on Coiled Tubing Operations & Slimhole Drilling Practices, Mar. 1-4, 1993, served by Global Tubing, LLC on Apr. 12, 2021 as Nos. GT0011300-GT0011313 in *Global Tubing, LLC vs. Tenaris Coiled Tubes, LLC et al.*, case No. 4:17-cv-03299 in the United States District Court for the Southern District of Texas, Houston Division, 14 pages.
- API Specification, "ISO 11960:2011 Petroleum and Natural Gas Industries Steel Pipes for Use as Casing or Tubing for Wells", published Jun. 2011, served by Global Tubing, LLC on Apr. 12, 2021 as Nos. GT0011314-GT0011404 in *Global Tubing, LLC vs. Tenaris Coiled Tubes, LLC et al.*, case No. 4:17-cv-03299 in the United States District Court for the Southern District of Texas, Houston Division, 91 pages.
- Afghoul et al., "Coiled Tubing: The Next Generation", published in 2004, served by Global Tubing, LLC on Apr. 12, 2021 as Nos. GT0011405-GT0011424, in *Global Tubing, LLC vs. Tenaris Coiled Tubes, LLC et al.*, case No. 4:17-cv-03299 in the United States District Court for the Southern District of Texas, Houston Division, 20 pages.
- U.S. Pat. No. 8,414,715, dated Apr. 9, 2013, served by Global Tubing, LLC on Apr. 12, 2021 as Nos. GT0011425-GT0011441 in *Global Tubing, LLC vs. Tenaris Coiled Tubes, LLC et al.*, case No. 4:17-cv-03299 in the United States District Court for the Southern District of Texas, Houston Division, 17 pages.
- U.S. Pat. No. 8,636,856, dated Jan. 28, 2014, served by Global Tubing, LLC on Apr. 12, 2021 as Nos. GT0011442-GT0011459 in *Global Tubing, LLC vs. Tenaris Coiled Tubes, LLC et al.*, case No. 4:17-cv-03299 in the United States District Court for the Southern District of Texas, Houston Division, 18 pages.
- English translation of JP2010270394A to Asano et al., Dec. 2, 2010, served by Global Tubing, LLC on Apr. 12, 2021 as Nos. GT0011542-GT0011546 in *Global Tubing, LLC vs. Tenaris Coiled Tubes, LLC et al.*, case No. 4:17-cv-03299 in the United States District Court for the Southern District of Texas, Houston Division, 5 pages.
- JP 2010-270394 A, Dec. 2, 2010, served by Global Tubing, LLC on Apr. 12, 2021 as Nos. GT0011547-GT0011555 in *Global Tubing, LLC vs. Tenaris Coiled Tubes, LLC et al.*, case No. 4:17-cv-03299 in the United States District Court for the Southern District of Texas, Houston Division, 9 pages.
- ASTM Designation: A 606-75, "American Society for Testing and Materials" American National Standards Institute publication date unknown, served by Global Tubing, LLC on Apr. 12, 2021 as Nos. GT0011556-GT0011559, in *Global Tubing, LLC vs. Tenaris Coiled Tubes, LLC et al.*, case No. 4:17-cv-03299 in the United States District Court for the Southern District of Texas, Houston Division, 4 pages.
- ASTM Designation: A 607-75 (Reapproved 1981), Standard Specification for Steel Sheet and Strip, Hot-Rolled and Cold-Rolled, High-Strength, Low-Alloy Columbium and/or Vanadium, publication date unknown, served by Global Tubing, LLC on Apr. 12, 2021 as Nos. GT0011560-GT0011563 in *Global Tubing, LLC vs. Tenaris Coiled Tubes, LLC et al.*, case No. 4:17-cv-03299 in the United States District Court for the Southern District of Texas, Houston Division, 4 pages.
- ASTM Designation: A 715-81, Standard Specification for Steel Sheet and Strip, Hot-Rolled and Cold-Rolled, High-Strength, Low-Alloy with Improved Formability, publication date unknown, served by Global Tubing, LLC on Apr. 12, 2021 as Nos. GT0011564-GT0011567, in *Global Tubing, LLC vs. Tenaris Coiled Tubes, LLC et al.*, case No. 4:17-cv-03299 in the United States District Court for the Southern District of Texas, Houston Division, 4 pages.
- Babu et al., "Effect of Austenitizing Temperature and Cooling Rate on the Structure and Properties of a Ultrahigh Strength Low Alloy Steel", 2006, served by Global Tubing, LLC on Apr. 12, 2021 as Nos. GT0011568-GT0011577, in *Global Tubing, LLC vs. Tenaris Coiled Tubes, LLC et al.*, case No. 4:17-cv-03299 in the United States District Court for the Southern District of Texas, Houston Division, 10 pages.
- Bhadeshia, "Martensite and Bainite in Steels: Transformation Mechanism and Mechanical Properties", Jan. 1997, served by Global Tubing, LLC on Apr. 12, 2021 as Nos. GT0011578-GT0011588, in *Global Tubing, LLC vs. Tenaris Coiled Tubes, LLC et al.*, case No. 4:17-cv-03299 in the United States District Court for the Southern District of Texas, Houston Division, 11 pages.
- Caballero et al., "The Microstructure of Continuously Cooled Tough Bainitic Steels", publication date unknown, served by Global Tubing, LLC on Apr. 12, 2021 as Nos. GT0011589-GT0011598 in *Global Tubing, LLC vs. Tenaris Coiled Tubes, LLC et al.*, case No. 4:17-cv-03299 in the United States District Court for the Southern District of Texas, Houston Division, 10 pages.
- Caballero et al., "Influence of bainite morphology on impact toughness of continuously cooled cementite free bainitic steels", publication date unknown, served by Global Tubing, LLC on Apr. 12, 2021 as Nos. GT0011599-GT0011606 in *Global Tubing, LLC vs. Tenaris Coiled Tubes, LLC et al.*, case No. 4:17-cv-03299 in the United States District Court for the Southern District of Texas, Houston Division, 8 pages.
- CLI International "Final Report: Serviceability of Coiled Tubing for Sour Oil and Gas Wells", publication date unknown, served by Global Tubing, LLC on Apr. 12, 2021 as Nos. GT0011607-GT0011796 in *Global Tubing, LLC vs. Tenaris Coiled Tubes, LLC et al.*, case No. 4:17-cv-03299 in the United States District Court for the Southern District of Texas, Houston Division, 190 pages.
- English translation of Chinese Patent No. 1873041A, Dec. 6, 2006, served by Global Tubing, LLC on Apr. 12, 2021 as Nos. GT0011821-GT0011827 in *Global Tubing, LLC vs. Tenaris Coiled Tubes, LLC et al.*, case No. 4:17-cv-03299 in the United States District Court for the Southern District of Texas, Houston Division, 7 pages.
- English translation of Chinese Patent No. 101603156A, Dec. 16, 2009, served by Global Tubing, LLC on Apr. 12, 2021 as Nos. GT0011842-GT0011854 in *Global Tubing, LLC vs. Tenaris Coiled Tubes, LLC et al.*, case No. 4:17-cv-03299 in the United States District Court for the Southern District of Texas, Houston Division, 13 pages.
- Cies, LP, "Coiled Tubing Manual", Rev. 72005-A, 2005, served by Global Tubing, LLC on Apr. 12, 2021 as Nos. GT0011855-GT0012788 in *Global Tubing, LLC vs. Tenaris Coiled Tubes, LLC et al.*, case No. 4:17-cv-03299 in the United States District Court for the Southern District of Texas, Houston Division, 934 pages.
- European Patent 2729590 B 1, Oct. 28, 2015, served by Global Tubing, LLC on Apr. 12, 2021 as Nos. GT0012789-GT0012802 in *Global Tubing, LLC vs. Tenaris Coiled Tubes, LLC et al.*, case No. 4:17-cv-03299 in the United States District Court for the Southern District of Texas, Houston Division, 14 pages.
- International Publication No. WO 2012/051335 A1, Apr. 19, 2012, served by Global Tubing, LLC on Apr. 12, 2021 as Nos. GT0012803-GT0012832 in *Global Tubing, LLC vs. Tenaris Coiled Tubes, LLC et al.*, case No. 4:17-cv-03299 in the United States District Court for the Southern District of Texas, Houston Division, 30 pages.
- U.S. Pat. No. 4,863,091, dated Sep. 5, 1989, served by Global Tubing, LLC on Apr. 12, 2021 as Nos. GT0012833-GT0012842 in *Global Tubing, LLC vs. Tenaris Coiled Tubes, LLC et al.*, case No. 4:17-cv-03299 in the United States District Court for the Southern District of Texas, Houston Division, 10 pages.
- U.S. Pat. No. 5,191,911, dated Mar. 9, 1993, served by Global Tubing, LLC on Apr. 12, 2021 as Nos. GT0012843-GT0012851 in *Global Tubing, LLC vs. Tenaris Coiled Tubes, LLC et al.*, case No. 4:17-cv-03299 in the United States District Court for the Southern District of Texas, Houston Division, 9 pages.
- U.S. Pat. No. 9,234,254, dated Jan. 12, 2016, served by Global Tubing, LLC on Apr. 12, 2021 as Nos. GT0012852-GT0012865 in *Global Tubing, LLC vs. Tenaris Coiled Tubes, LLC et al.*, case No. 4:17-cv-03299 in the United States District Court for the Southern District of Texas, Houston Division, 14 pages.

(56)

## References Cited

## OTHER PUBLICATIONS

- U.S. Pat. No. 9,708,681, dated Jul. 18, 2017, served by Global Tubing, LLC on Apr. 12, 2021 as Nos. GT0012866-GT0012878 in *Global Tubing, LLC vs. Tenaris Coiled Tubes, LLC et al.*, case No. 4:17-cv-03299 in the United States District Court for the Southern District of Texas, Houston Division, 13 pages.
- European Publication EP 2447386 A1, May 2, 2012, served by Global Tubing, LLC on Apr. 12, 2021 as Nos. GT0012879-GT0012903 in *Global Tubing, LLC vs. Tenaris Coiled Tubes, LLC et al.*, case No. 4:17-cv-03299 in the United States District Court for the Southern District of Texas, Houston Division, 25 pages.
- Mahallawi et al., "Influence of Heat Input and Post-Weld Heat Treatment on Boiler Steel P91 (9Cr-1Mo-V-Nb) Weld Joints, I. Microstructure", Mar. 2013, served by Global Tubing, LLC on Apr. 12, 2021 as Nos. GT0012904-GT0012913 in *Global Tubing, LLC vs. Tenaris Coiled Tubes, LLC et al.*, case No. 4:17-cv-03299 in the United States District Court for the Southern District of Texas, Houston Division, 10 pages.
- U.S. Pat. No. 2,586,041, dated Feb. 19, 1952, served by Global Tubing, LLC on Apr. 12, 2021 as Nos. GT0012914-GT0012915 in *Global Tubing, LLC vs. Tenaris Coiled Tubes, LLC et al.*, case No. 4:17-cv-03299 in the United States District Court for the Southern District of Texas, Houston Division, 2 pages.
- Johnson et al., "Toughness of Tempered Upper and Lower Bainitic Microstructures in a 4150 Steel", 1993, served by Global Tubing, LLC on Apr. 12, 2021 as Nos. GT0012916-GT0012924 in *Global Tubing, LLC vs. Tenaris Coiled Tubes, LLC et al.*, case No. 4:17-cv-03299 in the United States District Court for the Southern District of Texas, Houston Division, 9 pages.
- U.S. Pat. No. 6,267,828, dated Jul. 31, 2001, served by Global Tubing, LLC on Apr. 12, 2021 as Nos. GT0012967-GT0012977 in *Global Tubing, LLC vs. Tenaris Coiled Tubes, LLC et al.*, case No. 4:17-cv-03299 in the United States District Court for the Southern District of Texas, Houston Division, 11 pages.
- Lawrynowicz et al., "Features of Bainite Transformation in Steels", published Nov. 2002, served by Global Tubing, LLC on Apr. 12, 2021 as Nos. GT0012978-GT0013005 in *Global Tubing, LLC vs. Tenaris Coiled Tubes, LLC et al.*, case No. 4:17-cv-03299 in the United States District Court for the Southern District of Texas, Houston Division, 28 pages.
- Peet et al., "Fatigue of Extremely Fine Bainite", published in 2011 served by Global Tubing, LLC on Apr. 12, 2021 as Nos. GT0013042-GT0013046 in *Global Tubing, LLC vs. Tenaris Coiled Tubes, LLC et al.*, case No. 4:17-cv-03299 in the United States District Court for the Southern District of Texas, Houston Division, 5 pages.
- United States Publication No. 2011/0259482 A1, dated Oct. 27, 2011, served by Global Tubing, LLC on Apr. 12, 2021 as Nos. GT0013047-GT0013053 in *Global Tubing, LLC vs. Tenaris Coiled Tubes, LLC et al.*, case No. 4:17-cv-03299 in the United States District Court for the Southern District of Texas, Houston Division, 7 pages.
- U.S. Pat. No. 4,461,657, dated Jul. 24, 1984, served by Global Tubing, LLC on Apr. 12, 2021 as Nos. GT0013054-GT0013065 in *Global Tubing, LLC vs. Tenaris Coiled Tubes, LLC et al.*, case No. 4:17-cv-03299 in the United States District Court for the Southern District of Texas, Houston Division, 12 pages.
- SAE International, Surface Vehicle Standard J404, "Chemical Compositions of SAE Alloy Steels", Feb. 1991, served by Global Tubing, LLC on Apr. 12, 2021 as Nos. GT0013066-GT0013072 in *Global Tubing, LLC vs. Tenaris Coiled Tubes, LLC et al.*, case No. 4:17-cv-03299 in the United States District Court for the Southern District of Texas, Houston Division, 7 pages.
- Charbonnier et al., "Sulfide Stress Cracking of High Strength Modified Cr—Mo Steels", published May 1985, served by Global Tubing, LLC on Apr. 12, 2021 as Nos. GT0013073-GT0013082 in *Global Tubing, LLC vs. Tenaris Coiled Tubes, LLC et al.*, case No. 4:17-cv-03299 in the United States District Court for the Southern District of Texas, Houston Division, 10 pages.
- Craig, Bruce D., "Oilfield Metallurgy and Corrosion", Third Edition, published in 1993, served by Global Tubing, LLC on Apr. 12, 2021 as Nos. GT0013083-GT0013375 in *Global Tubing, LLC vs. Tenaris Coiled Tubes, LLC et al.*, case No. 4:17-cv-03299 in the United States District Court for the Southern District of Texas, Houston Division, 293 pages.
- Wang et al., "Study of High Strength Pipeline Steels with Different Microstructures", 2009, served by Global Tubing, LLC on Apr. 12, 2021 as Nos. GT0013376-GT0013382 in *Global Tubing, LLC vs. Tenaris Coiled Tubes, LLC et al.*, case No. 4:17-cv-03299 in the United States District Court for the Southern District of Texas, Houston Division, 7 pages.
- Rak et al., "Weldability and Toughness Assessment of Ti-Macroalloyed Offshore Steel", published Jan. 1997, served by Global Tubing, LLC on Apr. 12, 2021 as Nos. GT0013383-GT0013390 in *Global Tubing, LLC vs. Tenaris Coiled Tubes, LLC et al.*, case No. 4:17-cv-03299 in the United States District Court for the Southern District of Texas, Houston Division, 8 pages.
- Goodall, Graeme Robertson, "Welding High Strength Modern Line Pipe Steel", 2011, served by Global Tubing, LLC on Apr. 12, 2021 as Nos. GT0013391-GT0013603 in *Global Tubing, LLC vs. Tenaris Coiled Tubes, LLC et al.*, case No. 4:17-cv-03299 in the United States District Court for the Southern District of Texas, Houston Division, 213 pages.
- Cayard et al., "Serviceability of Coiled Tubing for Sour Oil and Gas Wells", 1996, served by Global Tubing, LLC on Apr. 12, 2021 as Nos. GT0013604-GT0013622 in *Global Tubing, LLC vs. Tenaris Coiled Tubes, LLC et al.*, case No. 4:17-cv-03299 in the United States District Court for the Southern District of Texas, Houston Division, 19 pages.
- Maurer Engineering Inc., "Coiled-Tubing Technology (1995-1998)", Apr. 1998, served by Global Tubing, LLC on Apr. 12, 2021 as Nos. GT0013623-GT0014082 in *Global Tubing, LLC vs. Tenaris Coiled Tubes, LLC et al.*, case No. 4:17-cv-03299 in the United States District Court for the Southern District of Texas, Houston Division, 460 pages.
- Cayard et al., "SPE 38410: Serviceability of Coiled Tubing for Sour Oil and Gas Wells", 1997, served by Global Tubing, LLC on Apr. 12, 2021 as Nos. GT0014083-GT0014097 in *Global Tubing, LLC vs. Tenaris Coiled Tubes, LLC et al.*, case No. 4:17-cv-03299 in the United States District Court for the Southern District of Texas, Houston Division, 15 pages.
- NACE International, NACE Standard TM0177-96 Item No. 21212, "Standard Test Method—Laboratory Testing of Metals for Resistance to Specific Forms of Environmental Cracking in H2S Environments", publication date unknown, served by Global Tubing, LLC on Apr. 12, 2021 as Nos. GT0014098-GT0014132 in *Global Tubing, LLC vs. Tenaris Coiled Tubes, LLC et al.*, case No. 4:17-cv-03299 in the United States District Court for the Southern District of Texas, Houston Division, 35 pages.
- NACE International, NACE Standard MR0175-93 Item No. 53024, "Standard Material Requirements—Sulfide Stress Cracking Resistant Metallic Materials for Oilfield Equipment", publication date unknown, served by Global Tubing, LLC on Apr. 12, 2021 as Nos. GT0014133-GT0014160 in *Global Tubing, LLC vs. Tenaris Coiled Tubes, LLC et al.*, case No. 4:17-cv-03299 in the United States District Court for the Southern District of Texas, Houston Division, 28 pages.
- Bramfitt et al., "Metallography and Microstructures of Carbon and Low-Alloy Steels", ASM Handbook, vol. 9: Metallography and Microstructures, 2004, served by Global Tubing, LLC on Apr. 12, 2021 as Nos. GT0014161-GT0014179 in *Global Tubing, LLC vs. Tenaris Coiled Tubes, LLC et al.*, case No. 4:17-cv-03299 in the United States District Court for the Southern District of Texas, Houston Division, 19 pages.
- U.S. Pat. No. 5,374,322, dated Dec. 20, 1994, served by Global Tubing, LLC on Apr. 12, 2021 as Nos. GT0022740-GT0022752 in *Global Tubing, LLC vs. Tenaris Coiled Tubes, LLC et al.*, case No. 4:17-cv-03299 in the United States District Court for the Southern District of Texas, Houston Division, 13 pages.
- United States Publication No. 2012/0199255 A1, dated Aug. 9, 2012, served by Global Tubing, LLC on Apr. 12, 2021 as Nos. GT0022819-GT0022846 in *Global Tubing, LLC vs. Tenaris Coiled*

(56)

## References Cited

## OTHER PUBLICATIONS

- Tubes, LLC et al.*, case No. 4:17-cv-03299 in the United States District Court for the Southern District of Texas, Houston Division, 28 pages.
- United States Publication No. 2005/0217768 A1, dated Oct. 6, 2005, served by Global Tubing, LLC on Apr. 12, 2021 as Nos. GT0022847-GT0022858 in *Global Tubing, LLC vs. Tenaris Coiled Tubes, LLC et al.*, case No. 4:17-cv-03299 in the United States District Court for the Southern District of Texas, Houston Division, 12 pages.
- Ruglic et al., "Normalizing of Steel", ASM Handbook, vol. 4, Heat Treating, publication date unknown, served by Global Tubing, LLC on Apr. 12, 2021 as Nos. GT0022892-GT0022902 in *Global Tubing, LLC vs. Tenaris Coiled Tubes, LLC et al.*, case No. 4:17-cv-03299 in the United States District Court for the Southern District of Texas, Houston Division, 11 pages.
- Ericsson, Torsten, "Principles of Heat Treating of Steels", ASM Handbook, vol. 4, Heat Treating, publication date unknown, served by Global Tubing, LLC on Apr. 12, 2021 as Nos. GT0022903-GT0022923 in *Global Tubing, LLC vs. Tenaris Coiled Tubes, LLC et al.*, case No. 4:17-cv-03299 in the United States District Court for the Southern District of Texas, Houston Division, 21 pages.
- Kirkaldy, J.S., "Quantitative Prediction of Transformation Hardening in Steels", ASM Handbook, vol. 4, Heat Treating, published in 1991, served by Global Tubing, LLC on Apr. 12, 2021 as Nos. GT0022924-GT0022940 in *Global Tubing, LLC vs. Tenaris Coiled Tubes, LLC et al.*, case No. 4:17-cv-03299 in the United States District Court for the Southern District of Texas, Houston Division, 17 pages.
- Bates, et al., "Quenching of Steel", ASM Handbook, vol. 4, Heat Treating, published in 1993, served by Global Tubing, LLC on Apr. 12, 2021 as Nos. GT0022941-GT0022998 in *Global Tubing, LLC vs. Tenaris Coiled Tubes, LLC et al.*, case No. 4:17-cv-03299 in the United States District Court for the Southern District of Texas, Houston Division, 58 pages.
- Canonica, Domenic A., "Stress-Relief Heat Treating of Steel", ASM Handbook, vol. 4, Heat Treating, publication date unknown, served by Global Tubing, LLC on Apr. 12, 2021 as Nos. GT0022999-GT0023004 in *Global Tubing, LLC vs. Tenaris Coiled Tubes, LLC et al.*, case No. 4:17-cv-03299 in the United States District Court for the Southern District of Texas, Houston Division, 6 pages.
- Welding Handbook, 9th Edition, vol. 4, Materials and Applications, Part 1, published 2011, served by Global Tubing, LLC on Apr. 12, 2021 as Nos. GT0023025-GT0023884 in *Global Tubing, LLC vs. Tenaris Coiled Tubes, LLC et al.*, case No. 4:17-cv-03299 in the United States District Court for the Southern District of Texas, Houston Division, 860 pages.
- Chitwood et al., "OTC 7032 High-Strength Coiled Tubing Expands Service Capabilities", 1992, served by Global Tubing, LLC on Apr. 12, 2021 as Nos. GT0023898-GT0023913 in *Global Tubing, LLC vs. Tenaris Coiled Tubes, LLC et al.*, case No. 4:17-cv-03299 in the United States District Court for the Southern District of Texas, Houston Division, 16 pages.
- Coiled Tubing Times, ISSN 1817-3330, Dec. 2012, served by Global Tubing, LLC on Apr. 12, 2021 as Nos. GT0024848-GT0024973 in *Global Tubing, LLC vs. Tenaris Coiled Tubes, LLC et al.*, case No. 4:17-cv-03299 in the United States District Court for the Southern District of Texas, Houston Division, 126 pages.
- International Coiled Tubing Association, "An Introduction to Coiled Tubing", 2004, served by Global Tubing, LLC on Apr. 12, 2021 as Nos. GT0024985-GT0025016 in *Global Tubing, LLC vs. Tenaris Coiled Tubes, LLC et al.*, case No. 4:17-cv-03299 in the United States District Court for the Southern District of Texas, Houston Division, 32 pages.
- English translation of Japanese Publication No. 2000-282144, Oct. 10, 2000, served by Global Tubing, LLC on Apr. 12, 2021 as Nos. GT0025063-GT0025073 in *Global Tubing, LLC vs. Tenaris Coiled Tubes, LLC et al.*, case No. 4:17-cv-03299 in the United States District Court for the Southern District of Texas, Houston Division, 11 pages.
- English translation of Japanese Publication No. S58-19439, Feb. 2, 1983, served by Global Tubing, LLC on Apr. 12, 2021 as Nos. GT0025074-GT0025083 in *Global Tubing, LLC vs. Tenaris Coiled Tubes, LLC et al.*, case No. 4:17-cv-03299 in the United States District Court for the Southern District of Texas, Houston Division, 10 pages.
- English translation of Chinese Publication No. 101602079 B, May 4, 2011, served by Global Tubing, LLC on Apr. 12, 2021 as Nos. GT0025109-GT0025131 in *Global Tubing, LLC vs. Tenaris Coiled Tubes, LLC et al.*, case No. 4:17-cv-03299 in the United States District Court for the Southern District of Texas, Houston Division, 23 pages.
- Makela, Weldon, "Heat Treating Basics", Jul. 26, 2012, served by Global Tubing, LLC on Apr. 12, 2021 as Nos. GT0025132-GT0025167 in *Global Tubing, LLC vs. Tenaris Coiled Tubes, LLC et al.*, case No. 4:17-cv-03299 in the United States District Court for the Southern District of Texas, Houston Division, 36 pages.
- U.S. Pat. No. 6,136,109, dated Oct. 24, 2000, served by Global Tubing, LLC on Apr. 12, 2021 as Nos. GT0025168-GT0025175 in *Global Tubing, LLC vs. Tenaris Coiled Tubes, LLC et al.*, case No. 4:17-cv-03299 in the United States District Court for the Southern District of Texas, Houston Division, 8 pages.
- United States Publication No. 2005/0034795 A1, dated Feb. 17, 2005, served by Global Tubing, LLC on Apr. 12, 2021 as Nos. GT0025176-GT0025187 in *Global Tubing, LLC vs. Tenaris Coiled Tubes, LLC et al.*, case No. 4:17-cv-03299 in the United States District Court for the Southern District of Texas, Houston Division, 12 pages.
- NACE International, NACE Standard MR0175-2002 Item No. 21304, "Standard Material Requirements—Sulfide Stress Cracking Resistant Metallic Materials for Oilfield Equipment", publication date unknown, served by Global Tubing, LLC on Apr. 12, 2021 as Nos. GT0025188-GT0025227 in *Global Tubing, LLC vs. Tenaris Coiled Tubes, LLC et al.*, case No. 4:17-cv-03299 in the United States District Court for the Southern District of Texas, Houston Division, 40 pages.
- NACE International, NACE Standard MR0175-2003 Item No. 21302, "Standard Material Requirements—Metals for Sulfide Stress Cracking and Stress Corrosion Cracking Resistance in Sour Oilfield Environments", publication date unknown, served by Global Tubing, LLC on Apr. 12, 2021 as Nos. GT0025228-GT0025271 in *Global Tubing, LLC vs. Tenaris Coiled Tubes, LLC et al.*, case No. 4:17-cv-03299 in the United States District Court for the Southern District of Texas, Houston Division, 44 pages.
- Ogden, Becky L., "Sulfide Stress Cracking—Practical Application to the Oil and Gas Industry", 2005, served by Global Tubing, LLC on Apr. 12, 2021 as Nos. GT0025272-GT0025286 in *Global Tubing, LLC vs. Tenaris Coiled Tubes, LLC et al.*, case No. 4:17-cv-03299 in the United States District Court for the Southern District of Texas, Houston Division, 15 pages.
- Canadian Publication No. CA 2414822 A1, Jun. 18, 2004, served by Global Tubing, LLC on Apr. 12, 2021 as Nos. GT0025287-GT0025322 in *Global Tubing, LLC vs. Tenaris Coiled Tubes, LLC et al.*, case No. 4:17-cv-03299 in the United States District Court for the Southern District of Texas, Houston Division, 36 pages.
- U.S. Pat. No. 7,048,811, dated May 23, 2006, served by Global Tubing, LLC on Apr. 12, 2021 as Nos. GT0025323-GT0025329 in *Global Tubing, LLC vs. Tenaris Coiled Tubes, LLC et al.*, case No. 4:17-cv-03299 in the United States District Court for the Southern District of Texas, Houston Division, 7 pages.
- Grossmann et al., "Principles of Heat Treatment—Fifth Edition", American Society for Metals, Apr. 1971, served by Global Tubing, LLC on Apr. 12, 2021 as Nos. GT0025330-GT0025645 in *Global Tubing, LLC vs. Tenaris Coiled Tubes, LLC et al.*, case No. 4:17-cv-03299 in the United States District Court for the Southern District of Texas, Houston Division, 316 pages.
- United States Publication No. 2008/0226491 A1, dated Sep. 19, 2008, served by Global Tubing, LLC on Apr. 12, 2021 as Nos. GT0025646-GT0025657 in *Global Tubing, LLC vs. Tenaris Coiled Tubes, LLC et al.*, case No. 4:17-cv-03299 in the United States District Court for the Southern District of Texas, Houston Division, 12 pages.

(56)

## References Cited

## OTHER PUBLICATIONS

- United States Publication No. 2008/0302452 A1, dated Dec. 11, 2008, served by Global Tubing, LLC on Apr. 12, 2021 as Nos. GT0025658-GT0025661 in *Global Tubing, LLC vs. Tenaris Coiled Tubes, LLC et al.*, case No. 4:17-cv-03299 in the United States District Court for the Southern District of Texas, Houston Division, 4 pages.
- U.S. Pat. No. 4,533,405, dated Aug. 6, 1985, served by Global Tubing, LLC on Apr. 12, 2021 as Nos. GT0025662-GT0025698 in *Global Tubing, LLC vs. Tenaris Coiled Tubes, LLC et al.*, case No. 4:17-cv-03299 in the United States District Court for the Southern District of Texas, Houston Division, 37 pages.
- U.S. Pat. No. 6,217,676, dated Apr. 17, 2001, served by Global Tubing, LLC on Apr. 12, 2021 as Nos. GT0025699-GT0025706 in *Global Tubing, LLC vs. Tenaris Coiled Tubes, LLC et al.*, case No. 4:17-cv-03299 in the United States District Court for the Southern District of Texas, Houston Division, 8 pages.
- English translation of Japanese Publication No. H06-116645, Apr. 26, 1994, served by Global Tubing, LLC on Apr. 12, 2021 as Nos. GT0025707-GT0025730 in *Global Tubing, LLC vs. Tenaris Coiled Tubes, LLC et al.*, case No. 4:17-cv-03299 in the United States District Court for the Southern District of Texas, Houston Division, 24 pages.
- English translation of Japanese Patent Publication No. H09-201688, Aug. 5, 1997, served by Global Tubing, LLC on Apr. 12, 2021 as Nos. GT0025731-GT0025748 in *Global Tubing, LLC vs. Tenaris Coiled Tubes, LLC et al.*, case No. 4:17-cv-03299 in the United States District Court for the Southern District of Texas, Houston Division, 18 pages.
- Turconi, et al., "Improvement of Resistance to SCC Initiation and Propagation of High Strength OCTG Through Microstructure and Precipitation Control", Paper No. 01077, Corrosion 2001, 2001, served by Global Tubing, LLC on Apr. 12, 2021 as Nos. GT0025769-GT0025783 in *Global Tubing, LLC vs. Tenaris Coiled Tubes, LLC et al.*, case No. 4:17-cv-03299 in the United States District Court for the Southern District of Texas, Houston Division, 15 pages.
- ASM International, Practical Heat Treating, Second Edition (#05144G), "Chapter 2—Fundamentals of the Heat Treating of Steel", 2006, served by Global Tubing, LLC on Apr. 12, 2021 as Nos. GT0035357-GT0035374 in *Global Tubing, LLC vs. Tenaris Coiled Tubes, LLC et al.*, case No. 4:17-cv-03299 in the United States District Court for the Southern District of Texas, Houston Division, 18 pages.
- Davis, J.R., Metals Handbook—Desk Edition, Second Edition, pp. 32, 61, 1471, 1517, and 103, published in 1998, served by Global Tubing, LLC on Apr. 12, 2021 as Nos. GT0051499-GT0051506 in *Global Tubing, LLC vs. Tenaris Coiled Tubes, LLC et al.*, case No. 4:17-cv-03299 in the United States District Court for the Southern District of Texas, Houston Division, 8 pages.
- Arai, et al., ASM Handbook, vol. 4—Heat Treating, 1994, served by Global Tubing, LLC on Apr. 12, 2021 as Nos. GT0130869-GT0131868 in *Global Tubing, LLC vs. Tenaris Coiled Tubes, LLC et al.*, case No. 4:17-cv-03299 in the United States District Court for the Southern District of Texas, Houston Division, 1000 pages.
- "SeaCAT LP—Specification for SeaCAT 100 Umbilical Tubing Continuous Anode Technology", <<http://seacatcorp.com/SeaCat100TubingSpecRev5Jul12003.htm>>, dated Nov. 14, 2004, served by Global Tubing, LLC on Apr. 12, 2021 as Nos. GT0210506-GT0210510 in *Global Tubing, LLC vs. Tenaris Coiled Tubes, LLC et al.*, case No. 4:17-cv-03299 in the United States District Court for the Southern District of Texas, Houston Division, 5 pages.
- "Specification for Coiled Tubing—U.S. Customary and SI Units", API Specification 5ST, First Edition, Apr. 2010, served by Global Tubing, LLC on Apr. 12, 2021 as Nos. GT0224055-GT0224129 in *Global Tubing, LLC vs. Tenaris Coiled Tubes, LLC et al.*, case No. 4:17-cv-03299 in the United States District Court for the Southern District of Texas, Houston Division, 75 pages.
- English translation of Chinese Publication No. CN 101898295 A, Dec. 1, 2010, served by Global Tubing, LLC on Apr. 12, 2021 as Nos. GT0283198-GT0283211 in *Global Tubing, LLC vs. Tenaris Coiled Tubes, LLC et al.*, case No. 4:17-cv-03299 in the United States District Court for the Southern District of Texas, Houston Division, 14 pages.
- ASTM International, Designation A 255-02, "Standard Test Methods for Determining Hardenability of Steel", publication date unknown, served by Global Tubing, LLC on Apr. 12, 2021 as Nos. GT0283245-GT0283268 in *Global Tubing, LLC vs. Tenaris Coiled Tubes, LLC et al.*, case No. 4:17-cv-03299 in the United States District Court for the Southern District of Texas, Houston Division, 24 pages.
- Newman, Kenneth R, SPE163884, "Development of a New CT Life Tracking Process", SPE International, 2013, served by Global Tubing, LLC on Apr. 12, 2021 as Nos. GT0283277-GT0283288 in *Global Tubing, LLC vs. Tenaris Coiled Tubes, LLC et al.*, case No. 4:17-cv-03299 in the United States District Court for the Southern District of Texas, Houston Division, 12 pages.
- Coloschi et al., SPE163930, "A Metallurgical Look at Coiled Tubing", SPE International, 2013, served by Global Tubing, LLC on Apr. 12, 2021 as Nos. GT0283289-GT0283297 in *Global Tubing, LLC vs. Tenaris Coiled Tubes, LLC et al.*, case No. 4:17-cv-03299 in the United States District Court for the Southern District of Texas, Houston Division, 9 pages.
- Seal et al., SPE 173660, "A Field Case History of Sulfate Reducing Bacteria Attack on Coiled Tubing Bias Welds—Root Causes and Remediation", SPE International, 2015, served by Global Tubing, LLC on Apr. 12, 2021 as Nos. GT0283298-GT0283313 in *Global Tubing, LLC vs. Tenaris Coiled Tubes, LLC et al.*, case No. 4:17-cv-03299 in the United States District Court for the Southern District of Texas, Houston Division, 16 pages.
- Padron et al., SPE-179045-MS, "CT100+ Bias Weld Fatigue Life Estimations—Are Adjustments Required", SPE International, 2016, served by Global Tubing, LLC on Apr. 12, 2021 as Nos. GT0283314-GT0283332 in *Global Tubing, LLC vs. Tenaris Coiled Tubes, LLC et al.*, case No. 4:17-cv-03299 in the United States District Court for the Southern District of Texas, Houston Division, 19 pages.
- Trzaska et al., "The calculation of CCT diagrams for engineering steels", Archives of Materials Science and Engineering, vol. 39, Issue 1, Sep. 2009, served by Global Tubing, LLC on Apr. 12, 2021 as Nos. GT0283333-GT0283340 in *Global Tubing, LLC vs. Tenaris Coiled Tubes, LLC et al.*, case No. 4:17-cv-03299 in the United States District Court for the Southern District of Texas, Houston Division, 8 pages.
- Saunders et al., "Using JMatPro to Model Materials Properties and Behavior", Dec. 2003, served by Global Tubing, LLC on Apr. 12, 2021 as Nos. GT0283341-GT0283346 in *Global Tubing, LLC vs. Tenaris Coiled Tubes, LLC et al.*, case No. 4:17-cv-03299 in the United States District Court for the Southern District of Texas, Houston Division, 6 pages.
- Zhao, J.-C., Methods for Phase Diagram Determination, published in 2011, served by Global Tubing, LLC on Apr. 12, 2021 as Nos. GT0283347-GT0283863 in *Global Tubing, LLC vs. Tenaris Coiled Tubes, LLC et al.*, case No. 4:17-cv-03299 in the United States District Court for the Southern District of Texas, Houston Division, 517 pages.
- Campbell, F.C., "Alloy Steels", Chapter 20, Elements of Metallurgy and Engineering Alloys, first printing Jun. 2008, served by Global Tubing, LLC on Apr. 12, 2021 as Nos. GT0283864-GT0283867 in *Global Tubing, LLC vs. Tenaris Coiled Tubes, LLC et al.*, case No. 4:17-cv-03299 in the United States District Court for the Southern District of Texas, Houston Division, 4 pages.
- API Specification 5L, Specification for Line Pipe, 45th Edition, Jul. 2013, served by Global Tubing, LLC on Apr. 12, 2021 as Nos. GT0283868-GT0284059 in *Global Tubing, LLC vs. Tenaris Coiled Tubes, LLC et al.*, case No. 4:17-cv-03299 in the United States District Court for the Southern District of Texas, Houston Division, 192 pages.
- ASTM International, Designation: E112-12, "Standard Test Methods for Determining Average Grain Size", publication date unknown, served by Global Tubing, LLC on Apr. 12, 2021 as Nos. GT0284060-GT0284086 in *Global Tubing, LLC vs. Tenaris Coiled Tubes, LLC et al.*, case No. 4:17-cv-03299 in the United States District Court for the Southern District of Texas, Houston Division, 27 pages.
- Gauthier, Michelle M., "Glossary of Terms", Engineered Materials Handbook Desk Edition, 1995, served by Global Tubing, LLC on

(56)

## References Cited

## OTHER PUBLICATIONS

- Apr. 12, 2021 as Nos. GT0284087-GT0284156 in *Global Tubing, LLC vs. Tenaris Coiled Tubes, LLC et al.*, case No. 4:17-cv-03299 in the United States District Court for the Southern District of Texas, Houston Division, 70 pages.
- Burner, Jr, Harold, "Hardenability of Carbon and Low-Alloy Steels", ASM Handbook, vol. 1: Properties and Selection: Irons, Steels, and High-Performance Alloys, 1990, served by Global Tubing, LLC on Apr. 12, 2021 as Nos. GT0284157-GT0284177 in *Global Tubing, LLC vs. Tenaris Coiled Tubes, LLC et al.*, case No. 4:17-cv-03299 in the United States District Court for the Southern District of Texas, Houston Division, 21 pages.
- "High-Strength Structural and High-Strength Low-Alloy Steels", ASM Handbook, vol. 1: Properties and Selection: Irons, Steels, and High-Performance Alloys, 1990, served by Global Tubing, LLC on Apr. 12, 2021 as Nos. GT0284178-GT0284212 in *Global Tubing, LLC vs. Tenaris Coiled Tubes, LLC et al.*, case No. 4:17-cv-03299 in the United States District Court for the Southern District of Texas, Houston Division, 35 pages.
- Kraus, George, "Microstructures, Processing, and Properties of Steels", ASM Handbook, vol. 1: Properties and Selection: Irons, Steels, and High-Performance Alloys, 1990, served by Global Tubing, LLC on Apr. 12, 2021 as Nos. GT0284213-GT0284226 in *Global Tubing, LLC vs. Tenaris Coiled Tubes, LLC et al.*, case No. 4:17-cv-03299 in the United States District Court for the Southern District of Texas, Houston Division, 14 pages.
- Liu et al., "Weldability of Steels", ASM Handbook vol. 1: Properties and Selection: Irons, Steels, and High-Performance Alloys, 1990, served by Global Tubing, LLC on Apr. 12, 2021 as Nos. GT0284227-GT0284237 in *Global Tubing, LLC vs. Tenaris Coiled Tubes, LLC et al.*, case No. 4:17-cv-03299 in the United States District Court for the Southern District of Texas, Houston Division, 11 pages.
- "Fracture Mechanics Properties of Carbon and Alloy Steels", ASM Handbook, vol. 19: Fatigue and Fracture, 1996, served by Global Tubing, LLC on Apr. 12, 2021 as No. GT0284238-GT0284278 in *Global Tubing, LLC vs. Tenaris Coiled Tubes, LLC et al.*, case No. 4:17-cv-03299 in the United States District Court for the Southern District of Texas, Houston Division, 41 pages.
- Landes, John D., "Fracture Toughness Testing", ASM Handbook, vol. 19: Fatigue and Fracture, 1996, served by Global Tubing, LLC on Apr. 12, 2021 as Nos. GT0284279-GT0284295 in *Global Tubing, LLC vs. Tenaris Coiled Tubes, LLC et al.*, case No. 4:17-cv-03299 in the United States District Court for the Southern District of Texas, Houston Division, 17 pages.
- Antolovich, Stephen D., "Alloy Design for Fatigue and Fracture", ASM Handbook, vol. 19: Fatigue and Fracture, 1996, served by Global Tubing, LLC on Apr. 12, 2021 as Nos. GT0284296-GT0284310 in *Global Tubing, LLC vs. Tenaris Coiled Tubes, LLC et al.*, case No. 4:17-cv-03299 in the United States District Court for the Southern District of Texas, Houston Division, 15 pages.
- "Software for Computational Materials Modeling and Simulation", ASM Handbook, vol. 22B, Metals Process Simulation, 2010, served by Global Tubing, LLC on Apr. 12, 2021 as Nos. GT0284311-GT0284318 in *Global Tubing, LLC vs. Tenaris Coiled Tubes, LLC et al.*, case No. 4:17-cv-03299 in the United States District Court for the Southern District of Texas, Houston Division, 8 pages.
- "Introduction to Steel Heat Treatment", ASM Handbook, vol. 4A, Steel Heat Treating Fundamentals and Processes, 2013, served by Global Tubing, LLC on Apr. 12, 2021 as Nos. GT0284319-GT0284341 in *Global Tubing, LLC vs. Tenaris Coiled Tubes, LLC et al.*, case No. 4:17-cv-03299 in the United States District Court for the Southern District of Texas, Houston Division, 23 pages.
- Chen et al., "Influence of Welding on Steel Weldment Properties", ASM Handbook, vol. 6: Welding, Brazing, and Soldering, 1993, served by Global Tubing, LLC on Apr. 12, 2021 as Nos. GT0284342-GT0284354 in *Global Tubing, LLC vs. Tenaris Coiled Tubes, LLC et al.*, case No. 4:17-cv-03299 in the United States District Court for the Southern District of Texas, Houston Division, 13 pages.
- Somers, Bruce R., "Introduction to the Selection of Carbon and Low-Alloy Steels", ASM Handbook, vol. 6: Welding, Brazing, and Soldering, 1993, served by Global Tubing, LLC on Apr. 12, 2021 as Nos. GT0284355-GT0284357 in *Global Tubing, LLC vs. Tenaris Coiled Tubes, LLC et al.*, case No. 4:17-cv-03299 in the United States District Court for the Southern District of Texas, Houston Division, 3 pages.
- Dupont, John N., "Fundamentals of Weld Solidification", ASM Handbook, vol. 6A, Welding Fundamentals and Processes, 2011, served by Global Tubing, LLC on Apr. 12, 2021 as Nos. GT0284358-GT0284376 in *Global Tubing, LLC vs. Tenaris Coiled Tubes, LLC et al.*, case No. 4:17-cv-03299 in the United States District Court for the Southern District of Texas, Houston Division, 19 pages.
- Maalekian, Mehran, "Solid-State Transformations in Weldments", ASM Handbook, vol. 6A, Welding Fundamentals and Processes, 2011, served by Global Tubing, LLC on Apr. 12, 2021 as Nos. GT0284377-GT0284400 in *Global Tubing, LLC vs. Tenaris Coiled Tubes, LLC et al.*, case No. 4:17-cv-03299 in the United States District Court for the Southern District of Texas, Houston Division, 24 pages.
- "Fracture Toughness and Fracture Mechanics", ASM Handbook, vol. 8: Mechanical Testing and Evaluation, 2000, served by Global Tubing, LLC on Apr. 12, 2021 as Nos. GT0284401-GT0284413 in *Global Tubing, LLC vs. Tenaris Coiled Tubes, LLC et al.*, case No. 4:17-cv-03299 in the United States District Court for the Southern District of Texas, Houston Division, 13 pages.
- "Impact Toughness Testing", ASM Handbook, vol. 8: Mechanical Testing and Evaluation, 2000, served by Global Tubing, LLC on Apr. 12, 2021 as Nos. GT0284414-GT0284429 in *Global Tubing, LLC vs. Tenaris Coiled Tubes, LLC et al.*, case No. 4:17-cv-03299 in the United States District Court for the Southern District of Texas, Houston Division, 16 pages.
- Revankar, Gopal, "Introduction to Hardness Testing", Mechanical Testing and Evaluation, vol. 8, ASM Handbook, revised online 2016, served by Global Tubing, LLC on Apr. 12, 2021 as Nos. GT0284430-GT0284442 in *Global Tubing, LLC vs. Tenaris Coiled Tubes, LLC et al.*, case No. 4:17-cv-03299 in the United States District Court for the Southern District of Texas, Houston Division, 13 pages.
- "Martensitic Structures", ASM Handbook, vol. 9: Metallography and Microstructures, 2004, served by Global Tubing, LLC on Apr. 12, 2021 as Nos. GT0284443-GT0284456 in *Global Tubing, LLC vs. Tenaris Coiled Tubes, LLC et al.*, case No. 4:17-cv-03299 in the United States District Court for the Southern District of Texas, Houston Division, 14 pages.
- Aliya, Debbie, "Physical Metallurgy Concepts in Interpretation of Microstructures", ASM Handbook, vol. 9: Metallography and Microstructures, 2004, served by Global Tubing, LLC on Apr. 12, 2021 as Nos. GT0284457-GT0284483 in *Global Tubing, LLC vs. Tenaris Coiled Tubes, LLC et al.*, case No. 4:17-cv-03299 in the United States District Court for the Southern District of Texas, Houston Division, 27 pages.
- Adams et al., SPE 29456, "An Evaluation of Large Diameter Coiled Tubing for Subsurface Production Tubulars", SPE International, 1995, served by Global Tubing, LLC on Apr. 12, 2021 as Nos. GT0284484-GT0284489 in *Global Tubing, LLC vs. Tenaris Coiled Tubes, LLC et al.*, case No. 4:17-cv-03299 in the United States District Court for the Southern District of Texas, Houston Division, 6 pages.
- U.S. Pat. No. 8,323,560, dated Dec. 4, 2012, served by Global Tubing, LLC on Apr. 12, 2021 as Nos. GT0284490-GT0284501 in *Global Tubing, LLC vs. Tenaris Coiled Tubes, LLC et al.*, case No. 4:17-cv-03299 in the United States District Court for the Southern District of Texas, Houston Division, 12 pages.
- Transcript of Videotaped Deposition of Philip Lewis, Dec. 15, 2020, as presented in *Global Tubing, LLC vs. Tenaris Coiled Tubes, LLC et al.*, case No. 4:17-cv-03299 in the United States District Court for the Southern District of Texas, Houston Division, 12 pages.
- Brown, et al., "DEA-97 Coiled Tubing Weld Cycle Life, Joint Industry Project", Part I: Final Project Report, Oct. 26, 1995, produced by Tenaris Coiled Tubes, LLC as Nos. TCT0282964-TCT0283071 in *Global Tubing, LLC vs. Tenaris Coiled Tubes, LLC et al.*, case No. 4:17-cv-03299 in the United States District Court for the Southern District of Texas, Houston Division, 108 pages.

(56)

**References Cited****OTHER PUBLICATIONS**

Southwestern Pipe, Inc, "The Development and Testing of Cymax 100 Coiled Tubing", Jan. 1992, produced by Tenaris Coiled Tubes, LLC as Nos. TCT0009962-TCT0009976 in *Global Tubing, LLC vs. Tenaris Coiled Tubes, LLC et al.*, case No. 4:17-cv-03299 in the United States District Court for the Southern District of Texas, Houston Division, 15 pages.

Southwestern Pipe, Inc, "Orbital Tig Welding, Cymax Coiled Tubing", Nov. 1992, produced by Tenaris Coiled Tubes, LLC as Nos. TCT0009977-TCT0009989 in *Global Tubing, LLC vs. Tenaris Coiled Tubes, LLC et al.*, case No. 4:17-cv-03299 in the United States District Court for the Southern District of Texas, Houston Division, 13 pages.

Southwestern Pipe, Inc, "Southwestern Pipe, Inc., Cymax Division, Coiled Tubing Specifications, Technical Data", Jan. 1, 1993, produced by Tenaris Coiled Tubes, LLC as Nos. TCT0009950-TCT0009961 in *Global Tubing, LLC vs. Tenaris Coiled Tubes, LLC et al.*, case No. 4:17-cv-03299 in the United States District Court for the Southern District of Texas, Houston Division, 12 pages.

CYMAX Southwestern Pipe, Inc. Presentation, publication date unknown, produced by Tenaris Coiled Tubes, LLC as Nos. TCT0013999-TCT0014057 in *Global Tubing, LLC vs. Tenaris Coiled Tubes, LLC et al.*, case No. 4:17-cv-03299 in the United States District Court for the Southern District of Texas, Houston Division, 57 pages.

Thompson, J.M., "Full Body Quenched and Tempered Coiled Tubing Theory vs. Field Experience", Cymax Division, published Mar. 1, 1994, produced by Tenaris Coiled Tubes, LLC as Nos. TCT0009930-TCT0009989 in *Global Tubing, LLC vs. Tenaris Coiled Tubes, LLC et al.*, case No. 4:17-cv-03299 in the United States District Court for the Southern District of Texas, Houston Division, 60 pages.

SeaCAT Corporation Specification for SeaCAT Umbilical Tubing Continuous Anode Technology, published in 2000, produced by Tenaris Coiled Tubes, LLC as Nos. TCT0373809-TCT0373819 in *Global Tubing, LLC vs. Tenaris Coiled Tubes, LLC et al.*, case No. 4:17-cv-03299 in the United States District Court for the Southern District of Texas, Houston Division, 11 pages.

SeaCAT 2001 Specification Umbilical Tubing Continuous Anode Technology, published Oct. 1, 2001—Revision 11, produced by Tenaris Coiled Tubes, LLC as Nos. TCT0372656-TCT0372661 in *Global Tubing, LLC vs. Tenaris Coiled Tubes, LLC et al.*, case No. 4:17-cv-03299 in the United States District Court for the Southern District of Texas, Houston Division, 6 pages.

SeaCAT Brochure—Coiled Tubing for Subsea Umbilical and Flowline Applications, publication date unknown, produced by Tenaris Coiled Tubes, LLC as Nos. TCT0375105-TCT0375246 in *Global Tubing, LLC vs. Tenaris Coiled Tubes, LLC et al.*, case No. 4:17-cv-03299 in the United States District Court for the Southern District of Texas, Houston Division, 142 pages.

SeaCAT Handbook—Coiled Tubing for Subsea Umbilical and Flowline Application, published in Spring 2005, produced by Tenaris Coiled Tubes, LLC as Nos. TCT0372486-TCT0372630 in *Global Tubing, LLC vs. Tenaris Coiled Tubes, LLC et al.*, case No. 4:17-cv-03299 in the United States District Court for the Southern District of Texas, Houston Division, 145 pages.

SeaCAT Shell Princess Project—published in Aug. 2002, produced by Tenaris Coiled Tubes, LLC as Nos. TCT0374261-TCT0374534 in *Global Tubing, LLC vs. Tenaris Coiled Tubes, LLC et al.*, case No. 4:17-cv-03299 in the United States District Court for the Southern District of Texas, Houston Division, 274 pages.

SeaCAT Process Control, published in 1999, produced by Tenaris Coiled Tubes, LLC as Nos. TCT0374535-TCT0374783 in *Global Tubing, LLC vs. Tenaris Coiled Tubes, LLC et al.*, case No. 4:17-cv-03299 in the United States District Court for the Southern District of Texas, Houston Division, 249 pages.

SeaCAT Qualification, published Oct. 4, 2001, produced by Tenaris Coiled Tubes, LLC as Nos. TCT0372729-TCT0372734 in *Global Tubing, LLC vs. Tenaris Coiled Tubes, LLC et al.*, case No.

4:17-cv-03299 in the United States District Court for the Southern District of Texas, Houston Division, 6 pages.

Auguston, Rogerio "The Influence of Chemical Composition and Microstructure of API Linepipe Steels on Hydrogen Induced Cracking and Sulfide Stress Corrosion Cracking", Materials Science and Engineering, published in 2003, produced by Tenaris Coiled Tubes, LLC as Nos. TCT0152051-TCT0152057 in *Global Tubing, LLC vs. Tenaris Coiled Tubes, LLC et al.*, case No. 4:17-cv-03299 in the United States District Court for the Southern District of Texas, Houston Division, 7 pages.

Faszold, J., SPE0153945 "Full-Scale Fatigue Testing with 130k Yield Tubing", SPE International, published in 2012, produced by Tenaris Coiled Tubes, LLC as Nos. TCT0626230-TCT0626235 in *Global Tubing, LLC vs. Tenaris Coiled Tubes, LLC et al.*, case No. 4:17-cv-03299 in the United States District Court for the Southern District of Texas, Houston Division, 6 pages.

Coulomb Status Summary Report published on Oct. 10, 2001, produced by Tenaris Coiled Tubes, LLC as Nos. TCT0372631-TCT0372667 in *Global Tubing, LLC vs. Tenaris Coiled Tubes, LLC et al.*, case No. 4:17-cv-03299 in the United States District Court for the Southern District of Texas, Houston Division, 37 pages.

Complaint filed by Global Tubing LLC (with Attachment: #1 Civil Cover Sheet) on Oct. 30, 2017, as pleading No. 1 in case 4:17-cv-03299, *Global Tubing, LLC vs. Tenaris Coiled Tubes, LLC et al.*, in the United States District Court for the Southern District of Texas, Houston Division.

First Amended Complaint with Jury Demand against Tenaris Coiled Tubes LLC filed by Global Tubing LLC on Feb. 12, 2018 as pleading No. 19 in case No. 4:17-cv-03299, *Global Tubing, LLC vs. Tenaris Coiled Tubes, LLC et al.*, in the United States District Court for the Southern District of Texas, Houston Division.

Answer to 19 Amended Complaint/Counterclaim/Crossclaim etc. by Tenaris Coiled Tubes LLC, filed on Aug. 13, 2018 as pleading No. 36 in case No. 4:17-cv-03299, *Global Tubing, LLC vs. Tenaris Coiled Tubes, LLC et al.*, in the United States District Court for the Southern District of Texas, Houston Division.

Supplement to 19 Amended Complaint/Counterclaim/Crossclaim etc., by Global Tubing LLC (with Attachments: #1 Exhibit 1, #2 Exhibit 2, #3 Exhibit 3, #4 Exhibit 4, #5 Exhibit 5) filed on Jan. 29, 2019 as pleading No. 47 in case No. 4:17-cv-03299, *Global Tubing, LLC vs. Tenaris Coiled Tubes, LLC et al.*, in the United States District Court for the Southern District of Texas, Houston Division. Amended Answer to 1 Complaint with Jury Demand, Counterclaim against Global Tubing LLC by Tenaris Coiled Tubes LLC (with Attachment: #1 Exhibit A), filed on Mar. 25, 2019 as pleading No. 57 in case No. 4:17-cv-03299, *Global Tubing, LLC vs. Tenaris Coiled Tubes, LLC et al.*, in the United States District Court for the Southern District of Texas, Houston Division.

Supplement to 57 Answer to Complaint, Counterclaim by Tenaris Coiled Tubes LLC filed on Jul. 9, 2019 as pleading No. 71 in case No. 4:17-cv-03299, *Global Tubing, LLC vs. Tenaris Coiled Tubes, LLC et al.*, in the United States District Court for the Southern District of Texas, Houston Division.

Second Amended Answer to 57 Answer to Complaint, Counterclaim with Jury Demand, Counterclaim against Global Tubing LLC by Tenaris Coiled Tubes, LLC, filed by Global Tubing, LLC (with Attachments: #1 Exhibit A, #2 Exhibit B, #3 Exhibit C) on Aug. 13, 2019 as pleading No. 74 in case No. 4:17-cv-03299, *Global Tubing, LLC vs. Tenaris Coiled Tubes, LLC et al.*, in the United States District Court for the Southern District of Texas, Houston Division.

Third Amended Answer to 74 Amended Answer, Counterclaim, with Jury Demand, Counterclaim against Global Tubing LLC by Tenaris S.A., Tenaris Coiled Tubes LLC (with Attachments: #1 Exhibit A, #2 Exhibit B, #3 Exhibit C) filed on Sep. 30, 2019 as pleading No. 76 in case No. 4:17-cv-03299, *Global Tubing, LLC vs. Tenaris Coiled Tubes, LLC et al.*, in the United States District Court for the Southern District of Texas, Houston Division.

Redaction to 80 Sealed Document by Global Tubing LLC [Redacted], filed by Global Tubing, LLC on Dec. 13, 2019 as pleading No. 97 in case No. 4:17-cv-03299, *Global Tubing, LLC vs. Tenaris Coiled Tubes, LLC et al.*, in the United States District Court for the Southern District of Texas, Houston Division.

(56)

## References Cited

## OTHER PUBLICATIONS

- Redaction to 81 Sealed Document by Global Tubing LLC, filed by Global Tubing, LLC on Jan. 23, 2020 as pleading No. 98 in case No. 4:17-cv-03299, *Global Tubing, LLC vs. Tenaris Coiled Tubes, LLC et al.*, in the United States District Court for the Southern District of Texas, Houston Division.
- Response to 96 Sealed Document Tenaris' Answer, Affirmative Defenses, and Counterclaims to Second Amended Complaint, filed by Global Tubing LLC on Jan. 31, 2020 as pleading No. 100 in case No. 4:17-cv-03299, *Global Tubing, LLC vs. Tenaris Coiled Tubes, LLC et al.*, in the United States District Court for the Southern District of Texas, Houston Division.
- Response to Tenaris Coiled Tubes, LLC's Amended Answer and Tenaris SA's Original Answer, Affirmative Defenses, and Counter-claims to Second Amended Complaint re: 119 Sealed Document [Redacted], filed by Global Tubing, LLC on Apr. 29, 2020 as pleading No. 124 in case No. 4:17-cv-03299, *Global Tubing, LLC vs. Tenaris Coiled Tubes, LLC et al.*, in the United States District Court for the Southern District of Texas, Houston Division.
- Tenaris' Supplemental Answer, Affirmative Defenses, and Counter-claims to Global Tubing's Second Amended Complaint [Redacted], filed by Tenaris Coiled Tubes, LLC and Tenaris S.A. (with #1 Appendix) on May 14, 2020 as pleading No. 129 in case No. 4:17-cv-03299, *Global Tubing, LLC vs. Tenaris Coiled Tubes, LLC et al.*, in the United States District Court for the Southern District of Texas, Houston Division.
- Memorandum and Order filed on Jun. 22, 2020 as pleading No. 140 in case No. 4:17-cv-03299, *Global Tubing, LLC vs. Tenaris Coiled Tubes, LLC et al.*, in the United States District Court for the Southern District of Texas, Houston Division.
- [No Author Listed], "Southwestern Pipe, Inc.—Cymax Coiled Tubing," Unknown if this document was publicly disclosed, but dated Jan. 1992, 1 page.
- Aggarwal, R. K., et al.: "Qualification of Solutions for Improving Fatigue Life at SCR Touch Down Zone", Deep Offshore Technology Conference, Nov. 8-10, 2005, Vitoria, Espirito Santo, Brazil, in 12 pages.
- Anelli, E., D. Colleuori, M. Pontremoli, G. Cumino, A Izquierdo, H. Quintanilla, "Metallurgical design of advanced heavy wall seamless pipes for deep-water applications", 4th International Conference on Pipeline Technology, May 9 to 13, 2004, Ostend, Belgium.
- Asahi, et al., Development of Ultra-high-strength Linepipe, X120, Nippon Steel Technical Report, Jul. 2004, Issue 90, pp. 82-87.
- ASM Handbook, Mechanical Tubing and Cold Finishing, Metals Handbook Desk Edition, (2000), 5 pages.
- ASTM A 182/A 182M "Standard Specification for Forged or Rolled Alloy and Stainless Steel Pipe Flanges, Forged Fittings, and Valves and Parts for High-Temperature Service."
- ASTM A 213/A 213M "Standard Specification for Seamless Ferritic and Austenitic Alloy-Steel Boiler, Superheater, and Heat-Exchanger Tubes."
- ASTM A336/A336M "Standard Specification for Alloy Steel Forgings for Pressure and High-Temperature Parts."
- ASTM A355 which is related to "Seamless Ferritic Alloy-Steel Pipe for High-Temperature Service".
- ASTM, "E112-13 Standard Test Methods for Determining Average Grain Size," ASTM International. 2012. p. 1-28.
- Bai, M., D. Liu, Y. Lou, X. Mao, L. Li, X. Huo, "Effects of Ti addition on low carbon hot strips produced by CSP process", Journal of University of Science and Technology Beijing, 2006, vol. 13, N° 3, p. 230.
- Beretta, Stefano et al., "Fatigue Assessment of Tubular Automotive Components in Presence of Inhomogeneities", Proceedings of IMECE2004, ASME International Mechanical Engineering Congress, Nov. 13-19, 2004, pp. 1-8.
- Berner, Robert A., "Tetragonal Iron Sulfide", Science, Aug. 31, 1962, vol. 137, Issue 3531, pp. 669.
- Berstein et al., "The Role of Traps in the Microstructural Control of Hydrogen Embrittlement of Steels" Hydrogen Degradation of Ferrous Alloys, Ed. T. Oriani, J. Hirth, and M. Smialowski, Noyes Publications, 1988, pp. 641-685.
- Bhadeshia et al., "Steels, Microstructure and Properties," Third Edition, Elsevier, Published in 2006, pp. 296.
- Boulegue, Jacques, "Equilibria in a sulfide rich water from Enghien-les-Bains, France", Geochimica et Cosmochimica Acta, Pergamon Press, 1977, vol. 41, pp. 1751-1758, Great Britain.
- Bruzzone et al., "Study of Hydrogen Permeation Through Passive Films on Iron Using Electrochemical Impedance Spectroscopy", PhD Thesis, 2003, Universidad Nacional del Comahue de Buenos Aires, Argentina (Abstract).
- Cancio et al., "Characterization of microalloy precipitates in the austenitic range of high strength low alloy steels", Steel Research, 2002, vol. 73, pp. 340-346.
- Carboni, A, A Pigani, G. Megahed, S. Paul, Casting and rolling of API X 70 grades for artic application in a thin slab rolling plane, Stahl u Eisen, 2008, N° 1, p. 131-134.
- Chang, L.C., "Microstructures and reaction kinetics of bainite transformation in Si-rich steels," XP0024874, Materials Science and Engineering, vol. 368, No. 1-2, Mar. 15, 2004, pp. 175-182, Abstract, Table 1.
- Clark, A Horrell, "Some Comments on the Composition and Stability Relations of Mackinawite", Neues Jahrbuch fur Mineralogie, 1966, vol. 5, pp. 300-304, London, England.
- Craig, Bruce D., "Effect of Copper on the Protectiveness of Iron Sulfide Films", Corrosion, National Association of Corrosion Engineers, 1984, vol. 40, Issue 9, pp. 471-474.
- D.O.T. 178.68 Spec. 39, pp. 831-840, Non reusable (non refillable) cylinders, Oct. 1, 2002.
- Davis, J.R., et al. "ASM—Speciality Handbook—Carbon and alloy steels" ASM Speciality Handbook, Carbon and Alloy Steels, 1996, pp. 12-27, XP002364757 US.
- De Medicis, Rinaldo, "Cubic FeS, A Metastable Iron Sulfide", Science, American Association For The Advancement of Science, Steen bock Memorial Library, Dec. 11, 1970, vol. 170, Issue 3963, pp. 723-728.
- Drill Rod Joint Depth Capacity Chart, downloaded Jan. 15, 2013; <http://www.boartlongyear.com/dri/11-rod-join-depth-capacity-chart>.
- E. Anelli, et al., "Metallurgical Design of Advanced Heavy Wall Seamless pipes for Deepwater Applications", 4th International Conference on Pipeline Technology, May 9-13, 2004, Ostend, Belgium.
- Echaniz, "The effect of microstructure on the KISSL of low alloy carbon steels", Nace Corrosion '98, EE. UU., Mar. 1998, pp. 22-27, San Diego.
- Echaniz, G., Morales, C., Perez, T., "Advances in Corrosion Control and Materials in Oil and Gas Production" Papers from Eurocorr 97 and Eurocorr 98, 13, P. S. Jackman and L. M. Smith, Published for the European Federation of Corrosion, No. 26, European Federation of Corrosion Publications, 1999.
- European Office Action in European Application No. 14159174.3 dated Sep. 16, 2016, 4 pages.
- European Search Report in European Application No. 14159174.3, dated Jul. 10, 2014, 5 pages.
- Extrait du Catalogue N 940, 1994.
- Fang, Hong-Sheng, et al.: "The Developing Prospect of Air-cooled Bainitic Steels", International Journal of Issi, vol. 2, No. 2, Feb. 1, 2005, pp. 9-18.
- Fratini et al.: "Improving friction stir welding of blanks of different thicknesses," Materials Science and Engineering A 459 (2007).
- Fritz T et al., "Characterization of electroplated nickel", Microsystem Technologies, Dec. 31, 2002, vol. 9, No. 1-2, pp. 87-91, Berlin, DE.
- Gojic, Mirko and Kosec, Ladislav, "The Susceptibility to the Hydrogen Embrittlement of Low Alloy Cr and CrMo Steels", ISIJ International, 1997, vol. 37, Issue 4, pp. 412-418.
- Gomez, G. et al.: "Air cooled bainitic steels for strong, seamless pipes—Part 1—allowy design, kinetics and microstructure", Materials Science and Technology, vol. 25, No. 12.

(56)

## References Cited

## OTHER PUBLICATIONS

- Heckmann, et al., Development of low carbon Nb—Ti—B microalloyed steels for high strength large diameter linepipe, Ironmaking and Steelmaking, 2005, vol. 32, Issue 4, pp. 337-341.
- Howells, et al.: "Challenges for Ultra-Deep Water Riser Systems", I IR, London, Apr. 1997, 11 pages.
- Hutchings et al., "Ratio of Specimen thickness to charging area for reliable hydrogen permeation measurement," British Corrosion Journal, 1993, vol. 28, Issue 4, pp. 309-312.
- Iino et al., "Aciers pour pipe-lines résistant au cloquage et au criquage dus à l'hydrogène", Revue de Metallurgie, 1979, vol. 76, Issue 8-9, pp. 591-609.
- Ikeda et al., "Influence of Environmental Conditions and Metallurgical Factors on Hydrogen Induced Cracking of Line Pipe Steel", Corrosion/SO, National Association of Corrosion Engineers, 1980, vol. 8, pp. 8/1-8/18, Houston, Texas.
- Izquierdo, et al.: "Qualification of Weldable X65 Grade Riser Sections with Upset Ends to Improve Fatigue Performance of Deepwater Steel Catenary Risers", Proceedings of the Eighteenth International Offshore and Polar Engineering Conference, Vancouver, BC, Canada, Jul. 6-11, 2008, p. 71.
- Jacobs, Lucinda and Emerson, Steven, "Trace Metal Solubility in an Anoxic Fjord", Earth and Planetary Sci. Letters, Elsevier Scientific Publishing Company, 1982, vol. 60, pp. 237-252, Amsterdam, Netherlands.
- Johnston, P.W., G.Brooks, "Effect of Al2O3 and TiO2 Additions on the Lubrication Characteristics of Mould Fluxes", Molten Slags, Fluxes and Salts 97 Conference, 1997 pp. 845-850.
- Kazutoshi Ohashi et al., "Evaluation of r-value of steels using Vickers hardness test", Journal of Physics: Conference Series, Aug. 7, 2012, p. 12045, vol. 379, No. 1, Institute of Physics Publishing, Bristol, GB.
- Keizer, Joel, "Statistical Thermodynamics of Nonequilibrium Processes", Springer-Verlag, 1987.
- Kishi, T., H.Takeucgi, M.Yamamiya, H.Tsuboi, T.Nakano, T.Ando, "Mold Powder Technology for Continuous Casting of Ti-Stabilized Stainless Steels", Nippon Steel Technical Report, No. 34, Jul. 1987, pp. 11-19.
- Korolev, D. F., "The Role of Iron Sulfides in the Accumulation of Molybdenum in Sedimentary Rocks of the Reduced Zone", Geochemistry, 1958, vol. 4, pp. 452-463.
- Lee, Sung Man and Lee, Jai Young, "The Effect of the Interface Character of TiC Particles on Hydrogen Trapping in Steel", Acta Metall., 1987, vol. 35, Issue 11, pp. 2695-2700.
- Mechanical Tubing and Cold Finishing, Metals Handbook Desk Edition, (2000), 5 pages.
- Mehling, Wilfred L.: "Hot Upset Forging," ASM Handbook vol. 14, 1998, pp. 84-95.
- Mishael, et al., "Practical Applications of Hydrogen Permeation Monitoring," Corrosion, Mar. 28-Apr. 1, 2004, Corrosion 2004, National Association of Corrosion Engineers, vol. Reprint No. 04476.
- Morice et al., "Moessbauer Studies of Iron Sulfides", J. Inorg. Nucl. Chem., 1969, vol. 31, pp. 3797-3802.
- Mukongo, T., P.C.Pistorius, and A.M.Garbers-Craig, "Viscosity Effect of Titanium Pickup by Mould Fluxes for Stainless Steel", Ironmaking and Steelmaking, 2004, vol. 31, No. 2, pp. 135-143.
- Mullet et al., "Surface Chemistry and Structural Properties of Mackinawite Prepared by Reaction of Sulfide Ions with Metallic Iron", Geochimica et Cosmochimica Acta, 2002, vol. 66, Issue 5, pp. 829-836.
- Murcowchick, James B. and Barnes, H.L., "Formation of a cubic FeS", American Mineralogist, 1986, vol. 71, pp. 1243-1246.
- NACE MR0175/ISO 15156-1 Petroleum and natural gas industries—Materials for use in H2S-containing Environments in oil and gas production—Part 1 : General principles for selection of crack-resistant materials, Jun. 28, 2007.
- Nagata, M., J. Speer, D. Matlock, "Titanium nitride precipitation behavior in thin slab cast high strength low alloyed steels", Metallurgical and Materials Transactions A, 2002, vol. 33A, p. 30993110.
- Nakai et al., "Development of Steels Resistant to Hydrogen Induced Cracking in Wet Hydrogen Sulfide Environment", Transactions of the ISIJ, 1979, vol. 19, pp. 401-410.
- Nandan et al.: "Recent advances in friction-stir welding—Process, weldment structure and properties," Progress in Materials Science 53 (2008) 980-1023.
- Pressure Equipment Directive 97/23/EC, May 29, 1997, downloaded from website: [http://ec.europa.eu/enterprise/pressure/equipment/ped/index\\_en.html](http://ec.europa.eu/enterprise/pressure/equipment/ped/index_en.html) on Aug. 4, 2010.
- Prevey, Paul, et al., "Introduction of Residual Stresses To Enhance Fatigue Performance in the Initial Design", Proceedings of Turbo Expo 2004, Jun. 14-17, 2004, pp. 1-9.
- Rickard, D.T., "The Chemistry of Iron Sulphide Formation at Low Temperatures", Stockholm Contrib. Geo I, 1969, vol. 26, pp. 67-95.
- Riecke, Ernst and Bohnenkamp, Konrad, "Über den Einfluss von Gittersoerstellen in Eisen auf die X-abs Wassersroffdiffusion", Z. Metallkde, 1984, vol. 75, pp. 76-81 (Abstract).
- Savatori et al. European Commission Report, EUR 2006, EUR2207, 3 pp. STN Abstract.
- Shanabarger, M.R. and Moorhead, R. Dale, "H2O Adsorption onto clean oxygen covered iron films", Surface Science, 1996, vol. 365, pp. 614-624.
- Shoemaker, et al., "Formation of Ferrous Monosulfide Polymorphs During Corrosion of Iron by Aqueous Hydrogen Sulfide at 21 degrees C", Journal of the Electrochemical Society, 1980, vol. 127, Issue 5, pp. 1007-1015.
- Skoczylas, G., A Dasgupta, R. Bommaraju, "Characterization of the chemical interactions during casting of High-titanium low carbon enameling steels", 1991 Steelmaking Conference Proceeding, pp. 707-717.
- Smyth, D., et al.: Steel Tubular Products, Properties and Selection: Irons, Steels, and High-Performance Alloys, vol. 1, ASM Handbook, ASM International, 1990, p. 327-336.
- Specification for Threading, Gauging and Thread Inspection of Casing, Tubing, and Line Pipe Threads, American Petroleum Institute, Specification 58, Apr. 2008, 15th Edition (Excerpts Only).
- Spry, Alan, "Metamorphic Textures", Pergamon Press, 1969, New York.
- Taira et al., "HIC and SSC Resistance of Line Pipes for Sour Gas Service", Nippon Kokan Technical Report, 1981, vol. 31, Issue 1-13.
- Taira et al., "Study on the Evaluation of Environmental Condition of Wet Sour Gas", Corrosion 83 (Reprint. No. 156, National Association of Corrosion Engineers), 1983, pp. 156/2-156/13, Houston, Texas.
- Takeno et al., "Metastable Cubic Iron Sulfide—With Special Reference to Mackinawite", American Mineralogist, 1970, vol. 55, pp. 1639-1649.
- Tenaris Newsletter for Pipeline Services, Apr. 2005, p. 1-8.
- Tenaris Newsletter for Pipeline Services, May 2003, p. 1-8.
- Thethi, et al.: "Alternative Construction for High Pressure High Temperature Steel Catenary Risers", OPT USA, Sep. 2003, p. 1-13.
- Thewlis, G., Weldability of X100 linepipe, Science and Technology of Welding and Joining, 2000, vol. 5, Issue 6, pp. 365-377.
- Tivelli et al., "Metallurgical Aspects of Heavy Wall—High Strength Seamless Pipes for Deep Water Applications", RioPipeline, Oct. 17-19, 2005, Rio, Brasil.
- Tivelli, M., G. Cumino, A Izquierdo, E. Anelli, A Di Schino, "Metallurgical Aspects of Heavy Wall—High Strength Seamless Pipes for Deep Water Applications", RioPipeline 2005, Oct. 17 to 19, 2005, Rio (Brasil), Paper n° IPB 1008 05.
- Todoroki, T. Ishii, K. Mizuno, A Hongo, "Effect of crystallization behavior of mold flux on slab surface quality of a Ti-bearing Fe—Cr—Ni super alloy cast by means of continuous casting process", Materials Science and Engineering A, 2005, vol. 413-414, p. 121-128.
- Turconi, G. L.: "Improvement of resistance to SSC initiation and propagation of high strength OCTG through microstructure and precipitation control"; "Paper 01077", NACE International, Houston, TX, Mar. 16, 2001. (XP009141583).
- Vaughan, D. J. and Ridout, M.S., "Moessbauer Studies of Some Sulphide Minerals", J. Inorg. Nucl. Chem., 1971, vol. 33, pp. 741-746.

(56)

**References Cited**

OTHER PUBLICATIONS

- Wegst, C.W., "Stahlussel", Auflage 1989, Seite 119, 2 pages.
- Yu, et al.: "New steels and alloys in mechanical engineering I ed.,"
- M: Mechanical Engineering, 1976, p. 19.
- "Seamless Steel Tubes for Pressure Purposes-Technical Delivery Conditions—Part 1: Non-alloy Steel Tubes with Specified Room Temperature Properties" British Standard BS EN 10216-1:2002 E:1-26, published May 2002.
- "Seamless Steel Tubes for Pressure Purposes-Technical Delivery Conditions—Part 2: Non-alloy and Alloy Steel Tubes with Specified Elevated Temperature Properties" British Standard BS EN 102162:2002+A2:2007: E: 1-45, published Aug. 2007.
- "Seamless Steel Tubes for Pressure Purposes—Technical Delivery Conditions—Part 3: Alloy Fine Grain Steel Tubes" British Standard BS EN 10216-3:2002 +A 1 :2004 E: 1-34, published Mar. 2004.
- "Seamless Steel Tubes for Pressure Purposes—Technical Delivery Conditions—Part 4: Non-alloy and Alloy Steel Tubes with Specified Low Temperature Properties" British Standard BS EN 10216-4:2002 + A 1 :2004 E: 1-30, published Mar. 2004.
- SDTX-4-17-CV-03299-222—Global Tubing—Order Granting Motion to Compel; Entered Mar. 26, 2021 USDC, SDTX; 30 pages.
- SDTX-4-17-CV-03299-471 Global Tubing—Order Denying Motion to Compel; Entered Sep. 9, 2022; USDC, SDTX; 10 pages.

\* cited by examiner



*FIG. 1*

FIG. 2





FIG. 3



FIG. 4



FIG. 5



FIG. 6

## METHOD OF FORMING AND HEAT TREATING COILED TUBING

### CROSS-REFERENCE TO RELATED APPLICATIONS

This application is a continuation of and claims the benefit of priority to U.S. patent application Ser. No. 14/872,490, filed Oct. 1, 2015, which is a divisional of U.S. patent application Ser. No. 13/229,517, now issued as U.S. Pat. No. 9,163,296 on Oct. 20, 2015, which claims the benefit of U.S. Provisional Application No. 61/436,156, filed Jan. 25, 2011, the entirety of each of which is hereby incorporated by reference.

### BACKGROUND OF THE INVENTION

#### Field of the Invention

Embodiments of the present disclosure are directed toward coiled tubes and methods of heat treating coiled tubes. Embodiments also relate to coiled tubes with tailored or varied properties along the length of the coiled tube.

#### Description of the Related Art

A coiled tube is a continuous length of tube coiled onto a spool, which is later uncoiled while entering service such as within a wellbore. Coiled tubes may be made from a variety of steels such as stainless steel or carbon steel. Coiled tubes can, for example, have an outer diameter between about 1 inch and about 5 inches, a wall thickness between about 0.080 inches and about 0.300 inches, and lengths up to about 50,000 feet. For example, typical lengths are about 15,000 feet, but lengths can be between about 10,000 feet to about 40,000 feet.

Coiled tubes can be produced by joining flat metal strips to produce a continuous length of flat metal that can be fed into a forming and welding line (e.g., ERW, Laser or other) of a tube mill where the flat metal strips are welded along their lengths to produce a continuous length of tube that is coiled onto a spool after the pipe exits the welding line. In some cases, the strips of metal joined together have different thickness and the coiled tube produced under this condition is called "tapered coiled tube" and this continuous tube has varying internal diameter due to the varying wall thickness of the resulting tube.

Another alternative to produce coiled tubes includes continuous hot rolling of tubes of an outside diameter different than the final outside diameter (e.g., U.S. Pat. No. 6,527,056 B2 describes a method producing coiled tubing strings in which the outer diameter varies continuously or nearly continuously over a portion of the string's length, WO2006/078768 describes a method in which the tubing exiting the tube mill is introduced into a forging process that substantially reduces the deliberately oversized outer diameter of the coil tubing in process to the nominal or target outer diameter, and EP 0788850 describes an example of a steel pipe-reducing apparatus, the entirety of each of which is hereby incorporated by reference, describe such tubes).

These methods described above produce coiled tube having constant properties since the tube is produced with the same material moving continuously through the same process. Therefore, the final design of the produced tube (e.g., dimension and properties) is a compromise between all the tube requirements while in service.

### SUMMARY

Described herein are coiled tubes with improved and varying properties along the length. In some embodiments, the coiled tubes may be produced by using a continuous and dynamic heat treatment process (CDHT). The resulting new product is a "composite" tube in the sense that the properties are not constant, generating a composite coiled tube (e.g., a continuous length of tube that can be coiled onto a spool for transport and uncoiled for use) with unique and optimized properties. The production of a continuous length of composite coil tube may be performed by introducing a previously produced spool of such product into a continuous and dynamic heat treatment line in order to generate a new material microstructure. The heat treatment is continuous because the tube moves through subsequent heating and cooling processes and it is dynamic because it can be modified to give a constantly changing heat treatment to different sections of the coiled tube.

Continuous coil tube may be made from shorter lengths of flat metal strip which are joined end-to-end, formed into tubular form, and seam welded to produce the starting coiled tube for the process are described herein. The starting coiled tube is thereafter introduced into a CDHT process. The CDHT modifies the microstructure thereby improving properties and minimizing heterogeneous properties between the tube body, the longitudinal weld, and the welds made to join the flat metal strips.

The heat treatment variables can be modified continuously in order to generate different mechanical properties, corrosion resistance properties, and/or microstructures along the length of the coiled tube. The resulting composite coiled tube could have localized increase in properties or selected properties in order to allow working at greater depths, localized increased stiffness to minimize buckling, increased corrosion resistance locally in the areas where exposure to higher concentrations of corrosive environments is expected, or any tailored design that has variation of properties in a specific location.

This variation of properties can result in a minimization or reduction of tapers, improving fatigue life, keeping the internal diameter constant for longer distances, minimizing unnecessary strip-to-strip welds, decreasing weight, improving inspection capabilities, tube volume and capacity among others. In particular, weight can be reduced by having an average wall thickness of the tube less than a tube with tapers since a tapered tube has increased wall thickness in certain regions such as the sections of tube at the top of a well. The outer diameter (OD) of the tapered tube typically remains constant while the inner diameter (ID) of the tube is changed to change the wall thickness. For example, an increase in wall thickness of a section of tube can decrease the ID of the section of tube. Therefore, a tube without tapering can have an ID that is substantially the same throughout the tube. By having a substantially constant ID, the ID along the entire length of tube can be inspected. For example, to inspect the ID, a drift ball can be used. However, the drift ball can only be used to inspect the smallest ID of the tapered tube. In addition, fluid flow rate through a tapered tube (e.g., capacity) is limited to the smallest ID of the tube. Therefore, by not reducing ID in certain sections of the tube by increasing wall thickness, the volume and capacity of the tube can be increased.

In certain embodiments, a method of treating a tube is provided. The method can include providing a spool of the tube, uncoiling the tube from the spool, heat treating the uncoiled tube to provide varied properties along a length of

the uncoiled tube, and coiling the tube after heat treating. The varied properties may include mechanical properties. At least one of temperature, soak time, heating rate, and cooling rate can be varied during heat treating of the uncoiled tube to provide varied properties along the length of the uncoiled tube. In certain embodiments, the tube is heat treated with two or more heat treatments (e.g., a double quench and tempering process). The tube may have a substantially constant wall thickness throughout the tube. The tube may have fewer changes in wall thickness as a result of the varied properties along the length of the tube in comparison to conventional tube without the varied properties to maintain sufficient properties for a particular application.

In certain embodiments, a coiled tube is provided. The coiled tube includes a first substantial portion of the tube having a first set of properties and a second substantial portion of the tube having a second set of properties such that at least one property of the first set of properties is different from at least one property of the second set of properties. For example, the difference between at least one property of the first set of properties and at least one property of the second set of properties can be larger than general variations in at least one property as a result of substantially similar steel composition with substantially similar heat treatment processing. At least one property of the first and second set of properties may include yield strength, tensile strength, fatigue life, corrosion resistance, grain size, or hardness. For example, the first substantial portion of the tube can include a first yield strength and the second substantial portion of the tube can include a second yield strength different (e.g., less or greater) than the first yield strength.

The tube may have fewer changes in wall thickness as a result of the varied properties along the length of the tube in comparison to conventional tube without the varied properties to maintain sufficient properties for a particular application. The tube may have a substantially constant wall thickness throughout the tube. Furthermore, the tube can have a substantially uniform composition throughout the tube. The tube may include a plurality of tube sections welded together and at least a portion of one of the tube sections of the plurality of tube sections comprises the first substantial portion and at least another portion of the same tube section comprises the second substantial portion.

In certain embodiments, a coiled tube for use in a well is provided. The coiled tube can include a continuous length of tube comprising a steel material having a substantially uniform composition along the entire length of the tube. The tube has at least a first portion configured to be positioned at the top of the well and at least a second portion configured to be positioned toward the bottom of the well relative to the first portion. The first portion of tube has a first yield strength and the second portion of tube has a second yield strength, the first yield strength can be different (e.g., greater or less) than the second yield strength. In some embodiments, the first portion has a yield strength greater than 100 ksi or about 100 ksi and the second portion has a yield strength less than 90 ksi or about 90 ksi. In further embodiments, the tube further includes a third portion of tube having a third yield strength between that of the first and second yield strength, the third portion being located between the first and second portions. However, the CDHT allows for the production of numerous combinations of properties (e.g. YS) for any length of pipe.

The tube can have a length of between 10,000 feet and 40,000 feet (or between about 10,000 feet and about 40,000 feet). The first portion of tube may have a length of between

1,000 feet (or about 1,000 feet) and 4,000 feet (or about 4,000 feet). Furthermore, the tube may include a plurality of tube sections welded together, and each of the tube sections may have a length of at least 1,500 feet (or about 1,500 feet). 5 The length of each tube section is related to the distance between bias welds to form the tube. The tube sections may be welded together after being formed into tubes or may be welded together as flat strips which are then formed into the tube. The tube may have a substantially constant wall thickness. For example, the first portion includes a first wall thickness and the second portion includes a second wall thickness that can be substantially the same as the first wall thickness. The first portion includes a first inner diameter and the second portion includes a second inner diameter that 10 can be substantially the same as the first inner diameter.

In some embodiments, the tube has an outer diameter between 1 inch and 5 inches (or between about 1 inch and about 5 inches). The tube may have a wall thickness between 0.080 inches and 0.300 inches (or between about 0.080 15 inches and about 0.300 inches). In further embodiments, the tube has a substantially constant wall thickness along the entire length of the tube. The tube may have a substantially constant inner diameter along the entire length of the tube. The tube may have no tapers in some embodiments, while in other embodiments, the tube has at least one taper.

#### BRIEF DESCRIPTION OF THE DRAWINGS

FIG. 1 illustrates an example coiled tube on a spool;  
30 FIG. 2 illustrates an example rig configured to coil and uncoil tube from a spool;

FIG. 3 illustrates an example of a continuous and dynamic heat treatment process;

FIG. 4 is a flow diagram of an embodiment of a method 35 of using a continuous and dynamic heat treatment process;

FIG. 5 is a plot of Rockwell C hardness (HRC) as a function of maximum temperature for tempering cycles which include heating and cooling at 40° C./sec and 1° C./sec, respectively; and

40 FIG. 6 is a plot of an example of required mechanical properties for a coiled tube as a function of depth from a well surface (0 ft) to a bottom of the well (22,500 ft) for a 110 ksi tube without being tapered, a four tapered 90 ksi tube, and a six tapered 80 ksi tube; also the dashed line shows mechanical properties for an embodiment of a composite tube without being tapered.

#### DETAILED DESCRIPTION

50 Described herein are coiled tubes having varying properties along the length of the coiled tube and methods of producing the same. In certain embodiments, a continuous and dynamic heat treatment process (CDHT) can be used to produce coiled tube with varying properties along the length 55 of the coiled tube. The heat treatment is continuous because the tube moves through subsequent heating and cooling processes, and the heat treatment is dynamic because it can be modified to give a constantly changing heat treatment to different sections of the coiled tube.

60 The heat treatment variables can be modified continuously in order to generate different mechanical properties along the length of the coiled tube. The resulting composite coiled tube can have at least a first portion of the tube having a first set of properties and a second portion of the tube having a second set of properties such that at least one property of the first set of properties is different from at least one property of the second set of properties.

In many applications, the coiled tube will be hanging inside a well and the coiled tube should be strong enough to support the associated axial loads; in other applications, the coiled tube will be pushed inside a well and when removed, the coiled tube will be pulled against the friction forces inside the well. In these examples, the material of the coiled tube on the top of the well will be subjected to the maximum axial load. In addition, for a deeper well, the wall thickness on the upper part of the coiled tube may be increased in order to withstand the axial load (both from hanging or pulling).

The use of tapered tubes has been used to allow increasing wall thickness only in the upper part of the coiled tube in order to reduce the total weight of the coiled tube. Materials of different compositions with higher mechanical properties have also been used in order to increase the resistance of the axial load, but these materials tend to be more expensive, more difficult to process, and have lower corrosion resistance.

In other applications, the coiled tube is pushed inside the well and there may be a requirement for increased stiffness; then the specification for the tube may require increased mechanical properties in order to maximize the stiffness of the coiled tube. In other cases, some areas of the well experience different temperatures and corrosive environments, and the coiled tube is specified with resistance to corrosive environments. Increased corrosion resistance can be produced by decreasing other material properties such as mechanical properties, which is contrary to the objective of increase axial resistance and stiffness.

Coiled tube is used by service companies that will provide a service in one location and then remove the coiled tube, recoil it and move it to a different location. FIG. 1 illustrates an example coiled tube 12 on a spool 14, and FIG. 2 illustrates an example rig 10 that can coil and un-coil coiled tube 12 on a spool 14 and direct the tube 12 into a well. The performance and fatigue life of the tube is related to low cycle fatigue associated with the coiling and un-coiling of the tube in each service operation. The fatigue life is usually reduced in the areas where the flat metal was originally joined. Also, the fatigue life is affected by the mechanical properties and operative conditions of the welding process.

Described herein is a product in which, by a special process, the coiled tube can be produced as a "composite" tube, in which the best properties for each section of the coiled tube are targeted. In this way, the tube properties are tailored along the length of the tube to generate the desired properties in the right place resulting in an overall increase of life due to fatigue, increase in corrosion resistance, and minimization of weight.

The special process (e.g., CDHT) takes advantage of the fact that material properties can be varied with appropriate heat treatments. Since a heat treatment is basically combinations of temperature and time, in a continuous heat treatment process, the temperature and speed (including heating and cooling rates) could be dynamically varied in order to modify the final properties of virtually every section of the tube being treated. Another advantage of the process is that since the final properties are affected by the final temperature and time cycle, the properties of the coiled tube could be fixed (e.g., repaired) if there has been a problem during the process, the heat treatment could be used to refurbish already used coiled tube if severe but reversible damage had occurred, or the heat treatment could be used to change properties of already produced coiled tube. This type of treatment allows the service companies to specify the best coiled tube for a given operation regardless of the number of wells the coiled tube is planned to operate in. If the tailored

coiled tube does not find more wells to service and it is obsolete (e.g., the coiled tube does not have properties for available applications), its properties could be changed provided there is no irreversible damage to the coiled tube.

5 In this way, the process (e.g., CDHT) described herein can generate a unique product (e.g., coiled tube) that could act as new product, new process for operation, and a new service. For example, the unique product can open up the possibility for a new "service" for repairing old coiled tubes or changing properties.

In certain embodiments, a method of treating a tube includes providing a spool of the tube, uncoiling the tube from the spool, heat treating the uncoiled tube to provide varied properties along a length of the uncoiled tube, and 15 coiling the tube after heat treating. FIG. 3 is a schematic that illustrates one embodiment. Tube 12 is uncoiled from a first spool 14a. After being uncoiled, the tube 12 goes through a CDHT process represented by box 20 and is then re-coiled on a second spool 14b.

20 In certain embodiments, the varied properties include mechanical properties. For example, the mechanical properties can include yield strength, ultimate tensile strength, elastic modulus, toughness, fracture toughness, hardness, grain size, fatigue life, fatigue strength. Many mechanical 25 properties are related to one another such as fracture toughness, hardness, fatigue life, and fatigue strength are related to tensile properties.

The varied properties may include corrosion resistance. Corrosion resistance can include sulfide stress cracking 30 (SSC) resistance. Hydrogen sulfide (H<sub>2</sub>S) dissolves in fluid (e.g., H<sub>2</sub>O), and the corrosive environment can be measured by pH and the amount of H<sub>2</sub>S in solution. Generally, the higher the pressure, the more H<sub>2</sub>S can be in solution. Temperature may also have an effect. Therefore, deeper 35 locations in the well experience higher pressure and higher H<sub>2</sub>S concentrations. As such, corrosion resistance of the tube can be increased along the length of the tube toward the section of tube at the bottom of the well. For example, about the bottom 75% of the well generally has the worst corrosive environment. Therefore, in certain embodiments, the bottom 75% of the length of tube has lower mechanical properties and hence higher corrosion resistance properties than the top 25% of the length of tube.

In general, corrosion resistance is related to mechanical 45 properties. For example, international standard NACE MR0175/ISO 155156 "Petroleum and natural gas industries—Materials for use in H<sub>2</sub>S-containing environments in oil and gas production" in Appendix A (A.2.2.3 for Casing and Tubing), the entirety of which is hereby incorporated by reference, shows a direct correlation of corrosion resistance to mechanical properties. In particular, Appendix A lists some materials that have given acceptable performance for resistance to SSC in the presence of H<sub>2</sub>S, under the stated metallurgical, environmental and mechanical conditions 55 based on field experience and/or laboratory testing. Appendix A indicates that as severity of the environment increases from region 1 to region 3 (increase H<sub>2</sub>S partial pressure and/or pH decreases), the recommendation for maximum yield strength (YS) decreases. For example, for region 1 of low severity YS<130 ksi (HRC<30), for region 2 of medium severity YS<110 ksi (HRC<27) and for region 3 of high severity (HRC<26 or maximum API5CT grade is T95 with HRC<25.4), suitable recommended material in all regions can be Cr—Mo quench and tempered steels.

60 Table I compares a standard steel product used for a coiled tube that has a ferrite and pearlite microstructure and varying grain size with steel that is quench and tempered.

Corrosion resistance of the quench and tempered steel is better than the standard product due to the uniformity of microstructure. Corrosion resistance of 80 ksi to 110 ksi coiled tube decreases as indicated, for example, in ISO 15156.

sulfur, 0.010 to 0.025 wt. % (or about 0.010 to about 0.025 wt. %) titanium, 0.0010 to 0.0025 wt. % (or about 0.0010 to about 0.0025 wt. %) boron, less than 0.0080 wt. % (or about 0.0080 wt. %) N and a ratio of Ti to N greater than 3.4 (or about 3.4); and

TABLE I

|                                     | Grade 80<br>(YS ~ 85 ksi) | Grade 90<br>(YS ~ 95 ksi)                                                                         | Grade 110<br>(YS ~ 115 ksi) | Corrosion Resistance<br>(due to microstructure) |
|-------------------------------------|---------------------------|---------------------------------------------------------------------------------------------------|-----------------------------|-------------------------------------------------|
| Product Type                        | Standard Product          | Ferrite + Pearlite + Bainite<br>Grain Size (GS) 80 > GS 90 > GS 110                               |                             | Low<br>(non-uniform<br>microstructure)          |
|                                     | Quench and Tempered       | Tempered Martensite<br>Carbide Size (CS) 80 > CS 90 > CS 110<br>Dislocation Density 80 < 90 < 110 |                             | High<br>(uniform<br>microstructure)             |
| Corrosion Resistance<br>(due to YS) | High                      | Medium                                                                                            | Low                         |                                                 |

During heat treatment, the microstructure will change from ferrite and pearlite to tempered martensite in the case of a quench and tempered process. A microstructure from a quench and tempered process is recommended by NACE for high strength pipes with SSC resistance. Also, carbide refinement due to tempering increases toughness. Localized hardness variations are reduced due to the elimination of pearlite or even bainite colonies that can result from segregation in as-rolled material. Localized increased hardness is detrimental for corrosion resistance. Fatigue life can also be increased by reduction of welds between sections of the tube, improving microstructure of the weld area through heat treatment, and/or reduction of mechanical properties.

A variety of steel compositions can be used in the methods described herein. Furthermore, various steel compositions can be used in the quench and temper process. Steel compositions can include, for example, carbon-manganese, chromium, molybdenum, boron and titanium, or a combination thereof. The steel composition may be selected based on, for example, the line speed, water temperature and pressure, product thickness, among others. Example steel compositions include:

Chromium bearing steel: the coiled tube comprising 0.23 to 0.28 wt. % (or about 0.23 to about 0.28 wt. %) carbon, 1.20 to 1.60 wt. % (or about 1.20 to about 1.60 wt. %) manganese, 0.15 to 0.35 wt. % (or about 0.15 to about 0.35 wt. %) silicon, 0.015 to 0.070 wt. % (or about 0.015 to about 0.070 wt. %) aluminum, less than 0.020 wt. % (or about 0.020 wt. %) phosphorus, less than 0.005 wt. % (or about 0.005 wt. %) sulfur, and 0.15 to 0.35 wt. % (about 0.15 to about 0.35 wt. %) chromium;

Carbon-Manganese: the coiled tube comprising 0.25 to 0.29 wt. % (or about 0.25 to about 0.29 wt. %) carbon, 1.30 to 1.45 wt. % (or about 1.30 to about 1.45 wt. %) manganese, 0.15 to 0.35 wt. % (or about 0.15 to about 0.35 wt. %) silicon, 0.015 to 0.050 wt. % (or about 0.015 to about 0.050 wt. %) aluminum, less than 0.020 wt. % (or about 0.020 wt. %) phosphorus, and less than 0.005 wt. % (or about 0.005 wt. %) sulfur;

Boron-Titanium: the coiled tube comprising 0.23 to 0.27 wt. % (or about 0.23 to about 0.27 wt. %) carbon, 1.30 to 1.50 wt. % (or about 1.30 to about 1.50 wt. %) manganese, 0.15 to 0.35 wt. % (or about 0.15 to about 0.35 wt. %) silicon, 0.015 to 0.070 wt. % (or about 0.015 to about 0.070 wt. %) aluminum, less than 0.020 wt. % (or about 0.020 wt. %) phosphorus, less than 0.005 wt. % (or about 0.005 wt. %)

<sup>20</sup> Martensitic Stainless Steel: the coiled tube comprising 0.12 wt. % (or about 0.12 wt. %) carbon, 0.19 wt. % (or about 0.19 wt. %) manganese, 0.24 wt. % (or about 0.24 wt. %) Si, 11.9 wt. % (or about 11.9 wt. %) chromium, 0.15 wt. % (or about 0.15 wt. %) columbium, 0.027 wt. % (or about 0.027 wt. %) molybdenum, less than 0.020 wt. % (or about 0.020 wt. %) phosphorus, and less than 0.005 wt. % (or about 0.005 wt. %) sulfur.

<sup>25</sup> Molybdenum could be added to the steel compositions above, and some steel compositions can be combined B—Ti—Cr to improve hardenability. Described in Example 1 in the below examples is a chromium bearing steel.

<sup>30</sup> In certain embodiments, at least one of temperature, soak time, heating rate, and cooling rate is varied during heat treating of the uncoiled tube to provide varied properties along the length of the uncoiled tube.

<sup>35</sup> In certain embodiments, the tube has fewer changes in wall thickness as a result of the varied properties along the length of the tube in comparison to conventional tube without the varied properties in order to maintain sufficient properties for a particular application. The tube may even have a substantially constant wall thickness throughout the tube (e.g., the tube has no tapers). The flat metal strips that are used to form tube sections of the tube can be, for example, between 1,500 feet and 3,000 feet (or about 1,500 feet and about 3,000 feet). Flat metal strips with smaller thickness may be longer than flat metal strips with larger thickness. However, if additional changes in wall thicknesses are desired, the flat metal strips may be shorter to allow for additional changes in wall thickness. Thus, if the length of the flat metal strip needed for each change in wall thickness is shorter than the possible maximum length of the flat metal strip, an extra weld joint is required. As previously discussed, additional weld joints can decrease fatigue life.

<sup>40</sup> <sup>50</sup> Therefore, as described herein, the number of weld joints can be decreased by minimizing the number of changes in wall thickness. For example, each tube section can have a length that is maximized. In certain embodiments, the tube does not have a tube section that is less than 1,500 feet long. In further embodiments, the average length of the tube sections is greater than 2,500 feet along the entire length of the tube. In further embodiments, the average length of tube sections is greater than if there were taper changes in the tube.

<sup>55</sup> <sup>60</sup> In certain embodiments, the starting coiled tube is unspooled at one end of the process, then it moves continuously through the heat treatment process and is spooled

again on the other end. The spooling devices can be designed to allow rapid changes in spooling velocity, and they can be moved to follow the coiled tube in order to change the spooling or un-spooling velocity in longitudinal units of tube per unit time even more rapidly (flying spooling).

The CDHT itself can include a series of heating and cooling devices that can easily change the heating and cooling rate of the material. In one example, the material is quenched and tempered dynamically, and FIG. 4 is an example flow diagram of the method 200. The method 200 can include quenching operations, intermediate operations, and tempering operations. In operational block 202, a coiled tube of a starting material is uncoiled. In operational block 204, the tube moves through a heating unit and then, in operational block 206, is quenched with water from the outside. The heating unit can modify the power in order to compensate for the changing mass flow when the tube's outer diameter and wall thickness changes, keeping productivity constant. It can also modify the power if the linear speed is changed when the tempering cycle is adjusted, keeping quenching temperatures constant but final properties different. In operational block 208, the tube can be dried.

The tempering operation can include a heating unit and a soaking unit. For example, in operational block 210, the tube can be tempered, and in operational block 212 the tube can be cooled. The stands of the soaking unit could be opened and ventilated so they can rapidly change the total length (e.g., time) of soaking, and at the same time, they can rapidly change the soaking temperature. At the exit of the soaking line, different air cooling devices can be placed in order to cool the tube to a coiling temperature at which there will not be further metallurgical changes. The control of the temperature and speed allows estimating the exact properties of the complete coiled tube, which is an advantage over certain conventional coiled tubes where testing is performed and properties can be only measured in the end of the spools. In certain conventional coiled tubes, the mechanical properties are estimated from less precise models for hot rolling at the hot rolled coil supplier as well as cold forming process during electrical resistive welding (ERW) forming. In operational block 214, the tube can be coiled onto a spool.

The resulting coiled tube can have a variety of configurations. In certain embodiments, a coiled tube includes a first substantial portion of the tube having a first set of properties, and a second substantial portion of the tube having a second set of properties such that at least one property of the first set of properties is different from at least one property of the second set of properties. Furthermore, the coiled tube may have more than two substantial portions. For example, the coiled tube may have a third substantial portion of tube which have a third set of properties such that at least one property of the third set is different from at least one property of the first set of properties and at least one property of the second set of properties. A substantial portion described herein may be a portion with a sufficient size (e.g., length) to enable measurement of at least one property of the portion. In certain embodiments, at least one property of the coiled tube varies continuously (e.g., near infinite number of portions).

In some embodiments, the first substantial portion of the tube has a first length between 1000 feet and 4000 feet (or between about 1,000 feet and about 4,000 feet), and the second substantial portion of the tube has a second length of at least 4000 feet (or at least about 4,000 feet). The first and second substantial portions may also have other various lengths.

In certain embodiments, at least one property of the first and second set of properties including yield strength, ultimate tensile strength, fatigue life, fatigue strength, grain size, corrosion resistance, elastic modulus, hardness, or any other properties described herein. Furthermore, a change of mechanical properties (e.g., yield strength) could allow a change in weight of the coiled tube.

In certain embodiments, the tube has fewer changes in wall thickness as a result in the varied properties along the 10 length of the tube in comparison to conventional tube without the varied properties in order to maintain sufficient properties for a particular application. The tube may even have a substantially constant wall thickness throughout the tube.

15 In certain embodiments, the tube has a substantially uniform composition throughout the tube. For example, the tube may have tube segments that were welded together that do not have significant differences in composition (e.g. tube segments with substantially similar composition). Tube segments can include either (1) tube segments that appear welded together since they were made by welding flat strips, formed into a tube, and welded longitudinally or (2) tube segments that are welded together after being formed into tubes and longitudinally welded.

20 25 30 35 40 45 50 55 60 65 70 75 80 85 90 95 100

In certain embodiments, the tube has a substantially uniform composition throughout the tube. For example, the tube may have tube segments that were welded together that do not have significant differences in composition (e.g. tube segments with substantially similar composition). Tube segments can include either (1) tube segments that appear welded together since they were made by welding flat strips, formed into a tube, and welded longitudinally or (2) tube segments that are welded together after being formed into tubes and longitudinally welded.

## EXAMPLES

The following examples are provided to demonstrate the benefits of the embodiments of the disclosed CDHT and resulting coiled tube. For example, as discussed below, coiled tube may be heat treated to provide coiled tube with overall unique properties. These examples are discussed for illustrative purposes and should not be construed to limit the scope of the disclosed embodiments.

### Example 1

As an example, a steel design that is quenched and tempered could include sufficient carbon, manganese and 40 could include chromium or molybdenum or combinations of boron and titanium, and be quenched and tempered at different temperatures. Various other steel compositions such as those described above can also be quenched and tempered in similar methods. In the example below, the coiled tube is comprised of about 0.23 to about 0.28 wt. % carbon, about 1.20 to about 1.60 wt. % manganese, about 0.15 to about 0.35 wt. % silicon, about 0.015 to about 0.070 wt. % aluminum, less than about 0.020 wt. % phosphorus, less than about 0.005 wt. % sulfur, and about 0.15 to about 0.35 wt. % chromium. The amount of each element is provided based upon the total weight of the steel composition.

Laboratory simulations and industrial trials were used to 55 measure the material response to quench and tempering cycles. The lengths were selected to guarantee uniform temperatures (more than 40 feet per condition, the material moved continuously through heating and cooling units in the industrial test and was stationary in the lab simulations). The material was subjected to tempering cycles of different 60 maximum temperatures by heating by induction at 40° C./sec up to the maximum temperature and then cooling in air at 1° C./sec (see FIG. 5 which shows the variation of hardness measured in Rockwell C scale (HRC) of the material as a function of maximum temperature). T1 in FIG. 65 5 is a reference temperature (about 1050° F. in this example) that results in a hardness of about 27.5 HRC. The reference temperature and resulting hardness can vary depending on

## 11

steel composition. These particular cycles did not have a soaking time at the maximum temperature (e.g. the material was not held at the maximum temperature for any significant time), but equivalent cycles at lower temperatures and for longer time could be applied. The material was previously water quenched to the same starting hardness level and to a microstructure composed of mainly martensite (more than 80% in volume).

By applying these tempering cycles, the final properties (e.g. yield strength) could be controlled from 80 to 140 ksi allowing the production of different final products. As indicated by the slope of the hardness as a function of temperature graph in FIG. 5, four points of hardness variation (approximately 11 ksi variation in tensile strength) can be produced if the maximum temperature is varied by more than 70° C. (e.g., hatched triangle in FIG. 5). The tensile strength is related to hardness, and discussion of the relationship can be found, for example, in Materials Science and Metallurgy, by H. Pollack, 4<sup>th</sup> edition, 1988, Prentice Hall, page 96, Table 3; shows that a 22.8 HRC is equivalent to 118 ksi and 26.6 HRC is equivalent to 129 ksi. A hardness difference of 3.8 HRC is 11 ksi in tensile strength. Certain other quench and tempered steels have also been observed to have a similar relationship. This temperature variation is much larger than the control capability of the tempering furnaces, and this example indicates that the tensile strength could be controlled at any point of the tube to much less than a 11 ksi variation. In a standard product without heat treatment, the mechanical properties variation along the length of a hot-rolled coil can be 11 ksi and between coils up to 15 ksi, so the mechanical properties of a standard product may vary along the length of the tube but in an uncontrolled way. In addition, in the standard product, these properties may vary as the tube is formed to different diameters; while in the case of the CDHT tubes these properties can remain constant with chemistry.

As demonstrated, the composite tube produced by a dynamic control of heat treatment process can have precisely selected properties that vary in a controlled fashion in each section of the tube. Calibration curves for the material used in this process allows controlling the exact properties at each location of the tubes by recording the temperature. Similar experiments on other compositions of tube can be used to create calibration curves which can then be used to create process parameters of the CDHT process to produce a coiled tube with select properties along the length of the tube. In addition, tempering models can be used to select processing conditions that could yield select properties along the length of the tube by varying parameters such as time and temperature. For example, Hollomon et al., "Time-temperature Relations in Tempering Steel," Transactions of the American Institute of Mining, 1945, pages 223-249, describes a classical tempering model approach. Hollomon describes that the final hardness after tempering of a well quenched material (high % of martensite) is a function of a time-temperature equation that varies with the type of steel. This model can be used to calculate the final hardness of a material after tempering for any combination of time and temperatures after generating some experimental data. The calibration curves for a tempering process can be generated after the model has been fitted with the experimental data.

In order to dynamically change the properties, the temperature can be increased rapidly or decreased rapidly using induction heating, air cooling or changing the soaking time (if the cycle of tempering uses temperature and a soaking time and not only temperature as is the case for the example in FIG. 5). This process can be used to generate a unique

## 12

coiled tube product with varying properties that are changed in order to optimize its use as shown in the examples below. The heat treated microstructure can be much more refined and homogeneous than the hot-rolled microstructure, which can provide improved corrosion and fatigue performance. The heat treatment can also relieve internal stresses of the material, which were generated during forming (e.g., hot-rolling and pipe forming).

## Example 2

In certain applications, a coiled tube may be required to operate in wells of up to 22,500 ft deep. The tube minimum wall thickness may be 0.134" and the tube OD may be 2.00". The material may also have good performance in H<sub>2</sub>S containing environments and good fatigue life.

If the tube is designed for axial load, without taper changes and with a safety factor of 70%, the material may have a Specified Minimum Yield Strength (SMYS) of at least 110 ksi:

$$0.70 \times \text{SMYS} = A(\text{area}) \times L(\text{length}) \times \text{Density} / A = L \times \text{Density}$$

$$\text{SMYS} = L \times \text{Density} / 0.70 = 22,500 \text{ ft} \times (0.283 \text{ lb/in}^3) \times (12 \text{ in/ft}) / 0.70$$

$$\text{SMYS} \approx 110,000 \text{ psi}$$

The density value was estimated as the density of iron of about 0.283 lb/in<sup>3</sup>. This indicates that if the tube is designed to have a yield strength of 110 ksi, the cross section at the top of the well will be capable of withstanding the weight of the coiled tube. If the same coiled tube is produced with material having a SMYS of 90 or 80 ksi, it may be necessary to taper the upper length of the coiled tube in order to increase the resistance area "A" (e.g. the wall thickness of the coiled tube is increased in the section closer to the well surface compared to the section of the coiled tube closer to the well bottom. FIG. 6 shows a full line (see the solid lines in FIG. 6) of the required mechanical properties from the bottom of the well (22,500 ft) to the well surface (0 ft) for a 110, 90 and 80 ksi coiled tube. As illustrated in FIG. 6, by performing wall thickness changes (e.g. tapers) (which are generally restricted to a number of standard thicknesses produced by the steel rolling mill), the resulting tapered coiled tube could be built with 110, 90 or 80 ksi material (when the whole coiled tube is manufactured in only one type of material).

If a composite coiled tube is defined with the properties varying as indicated by the dotted line in FIG. 6, the well could be serviced since the properties vary to improve the overall performance of the coiled tube as indicated in Table II below. The estimation of relative fatigue life and pumping pressure (calculated relative to the composite coiled tube) in Table II is defined based on models used for prediction of service life and current standards. For example, as illustrated in FIG. 6, the tube can have a yield strength of at least 110 ksi to a depth of about 4,000 feet, a yield strength of at least 90 ksi to a depth of about 6,500 feet and a yield strength of at least 80 ksi at depths greater than about 6,500 feet.

TABLE II

| Example               | # of taper changes | # of weld joints | Internal Flash Removal (Y/N) | Relative weight | Relative pumping pressure | Relative fatigue life | SSC resistance | Cost    |
|-----------------------|--------------------|------------------|------------------------------|-----------------|---------------------------|-----------------------|----------------|---------|
| 110 ksi coiled tube   | 0                  | 9                | Y                            | 100.0%          | 100.0%                    | 80.0%                 | Worst          | Highest |
| 90 ksi coiled tube    | 4                  | 11               | N                            | 103.1%          | 102.8%                    | 53.3%                 | Medium         | Medium  |
| 80 ksi coiled tube    | 7                  | 12               | N                            | 107.5%          | 107.5%                    | 48.9%                 | Best           | Medium  |
| Composite coiled tube | 0                  | 9                | Y                            | 100.0%          | 100.0%                    | 100.0%                | Best           | Lowest  |

Internal flash removal refers to the elimination of the material that is expelled from the weld during the ERW process. This material can only be removed if the taper changes are reduced to zero (e.g. taper changes can restrict or prevent the removal of flash). The presence of the flash can affect the fatigue life as well as the ability to inspect the tube.

The best coiled tube is the composite coiled tube because, while keeping the number of taper changes to zero and the tube weight to a minimum, it has lower mechanical properties down the coiled tube, improving the fatigue life as well as the resistance to embrittlement in H<sub>2</sub>S environments by SSC. Furthermore, the cost of the raw material for the composite coiled tube can be lower. An “all 80 ksi” coiled tube will have similar resistance to SSC but with 7.5% weight increase, while an “all 110 ksi” material will have similar weight and no taper changes but lower fatigue and SSC resistance.

In addition, the number of weld joints between tube sections can be minimized. As shown in Table II, the number of tube sections was higher for 90 ksi coiled tube and 80 ksi coiled tube because of the wall thickness changes (e.g., tapers). The additional tapers can reduce the fatigue resistance of the tube. In certain embodiments, the average length of the tube sections is greater than 2500 feet along the entire length of the tube. In further embodiments, the average length of tube sections is greater than if there were taper changes in the tube.

The composite coiled tube, by minimizing the number of tapers, also increases the coiled tube capacity and volume, as well as reliability of inspection, using a drift ball for example. The internal flash removal with no tapers is also possible if desired.

For a tapered coiled tube, the increased wall thickness reduces the inner diameter and results in higher pumping pressure for the same volumetric flow rate. Higher pumping pressure will both increase the energy required for pumping and reduce the fatigue life by increasing internal stresses. Therefore, the composite product described herein can have optimized properties and improved properties over a tapered coiled tube.

Pumping pressure can be a function of tube length and inside diameter, and pumping pressure can be calculated using well-known fluid mechanics relationships. Therefore, by increasing the inside diameter of the tube, the pumping pressure can be reduced for a certain flow rate. Furthermore, fatigue life can be affected by many factors including the tube yield strength, the internal pressure, and others. The example tubes described herein can have improved fatigue life by having a combined effect of selecting yield strength, decreasing internal pressure (e.g., pumping pressure), and decreasing number of strip to strip welds. SSC resistance can

15 be assessed in accordance with NACE TM0177 and NACE MR0175. One strong correlation in C—Mn steels is the relationship between hardness and SSC resistance. As previously discussed, in general, steel with a higher hardness results in lower SSC resistance. Also in general, steel with a higher strength has a higher hardness which results in a lower SSC resistance. The composite coiled tube can have lower strength tube confined to the lower part of the coiled tube where the SSC exposure is higher. Furthermore, the composite coiled tube can have high strength tube confined to the upper part of the coiled tube where the SSC exposure is less.

20 The properties after a heat treatment are affected by the time and temperature history of the material, making the process subject to validation. The validation process is supported by metallurgical models that allows for the correct prediction of tube properties at each section of the coiled tube. In the certain conventional coiled tubes, the properties along the length of the coiled tube depend on hot rolled schedule at the steel supplier, sequence of coil splicing (since not all coils are equal), as well as the cold forming process at tube mill. The composite heat treated coiled tube is much more reliable than the standard coiled tube. For example, the properties of the composite heat treated coiled tube can be more consistent since the properties primarily depend on the heat treatment process while conventional coiled tubes have many variables that result in large variations in properties between sections of the coiled tube and also between different coiled tubes.

25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635

## 15

overall performance of the coiled tube. These property variations could not be generated during the hot rolling since the property changes are affected by the degree of reduction during rolling.

## Example 4

During hot rolling, the final properties are affected by the schedule of reduction at the hot rolling mill as well as the cooling at the run out table and final coiling process. Since the water in the run out table could generate differing cooling patterns across the width of the hot rolled coil, a faster cooling on coil edges and variations along the length due to "hot lead end practices" to facilitate coiling, as well as differential cooling of the inside of the coil with respect to the ends, the properties of the tubes would inherit these variations. In the case of the heat treated coiled tubes, the variation of properties are mainly affected by the chemistry and hence occur at a heat level (e.g., a heat size is the size of the ladle in the steelmaking process and hence is the maximum volume with same chemistry produced by a batch steelmaking process). The variation of properties of the composite heat treated coiled tube could be under control by having improved control of the heat treatment (heating, soaking, cooling, etc. (e.g., rate and time)) along the length of the coiled tube.

Although the foregoing description has shown, described, and pointed out the fundamental novel features of the present teachings, it will be understood that various omissions, substitutions, and changes in the form of the detail of the apparatus as illustrated, as well as the uses thereof, may be made by those skilled in the art, without departing from the scope of the present teachings. Consequently, the scope of the present teachings should not be limited to the foregoing discussion.

## What is claimed is:

1. A method of forming and heat treating a coiled tube, the method comprising:  
 providing a plurality of steel strips to be welded together, each of the steel strips including from about 0.010 wt. % to about 0.025 wt. % titanium and from about 0.0010 wt. % to about 0.0025 wt. % of boron;  
 welding the plurality of steel strips together end-to-end to form a plurality of end-to-end welded strips and longitudinally welding the plurality of end-to-end welded strips to form a tube comprising:  
 a first tube section with a substantially constant inner diameter, outer diameter, and wall thickness; and a second tube section with a wall thickness that is different than the wall thickness of the first tube section;  
 after forming the tube, performing a continuous and dynamic heat treatment (CDHT) process comprising a continuous quench and temper heat treatment along the tube, wherein heating rate is modified to compensate for the change in wall thickness from the first tube section to the second tube section, thereby resulting in a tube with substantially uniform microstructure comprising at least 80% tempered martensite across (a) the plurality of steel strips, (b) the plurality of end-to-end welds joining the steel strips, and (c) the plurality of longitudinal welds joining the plurality of end-to-end welded steel strips; and  
 coiling the first portion of coiled tubing to form a coiled tube.

## 16

2. The method of claim 1, wherein the step of coiling the first portion of coiled tubing to form a coiled tube comprises coiling the first portion of coiled tubing on a spool.
3. The method of claim 1, further comprising:  
  - 5 after forming the first portion of coiled tubing, coiling the first portion of coiled tubing on a spool;
  - 10 uncoiling the first portion of coiled tubing from the spool prior to performing the CDHT process;
  - 15 performing the CDHT process; and
  - 20 after performing the CDHT process, re-coiling the first portion of coiled tubing.
4. The method of claim 1, wherein the plurality of steel strips have a substantially uniform steel composition.
5. The method of claim 1, wherein the first portion of coiled tubing has a tempered martensite microstructure along substantially its entire length.
6. The method of claim 1, wherein performing the continuous quench and temper heat treatment comprises translating the first portion of coiled tubing through a heat treatment system that performs heating action, cooling action, or both.
7. The method of claim 6, wherein translating the first portion of coiled tubing is at variable speeds.
8. The method of claim 1, wherein performing the continuous quench and temper heat treatment comprises at least one quenching operation, intermediate operation, and tempering operation.
9. The method of claim 1, wherein at least one parameter of the continuous quench and temper heat treatment is selected from a group consisting of temperature, soak time, heating rate, and cooling rate.
10. The method of claim 1, wherein at least one parameter of the continuous quench and temper heat treatment is selected from a group consisting of at least two of temperature, soak time, heating rate, and cooling rate.
11. The method of claim 1, wherein a yield strength of the first portion of coiled tubing is between 80 ksi and 140 ksi.
12. The method of claim 1, wherein the step of providing a plurality of steel strips to be welded together, comprises each of the steel strips including from about 1.30 wt. % to about 1.50 wt. % manganese.
13. The method of claim 1, further comprises providing a plurality of steel strips to be welded together, each of the plurality of steel strips including from about 0.15 wt. % to about 0.35 wt. % silicon.
14. The method of claim 1, further comprises providing a plurality of steel strips to be welded together, each of the plurality of steel strips including less than about 0.005 wt. % sulfur.
15. The method of claim 1, further comprises providing a plurality of steel strips to be welded together, each of the plurality of steel strips including from about 0.015 wt. % to about 0.070 wt. % aluminum.
16. The method of claim 1, further comprises providing a plurality of steel strips to be welded together, each of the plurality of steel strips including less than about 0.020 wt. % phosphorus.
17. The method of claim 1, further comprises providing a plurality of steel strips to be welded together, each of the steel strips including from about 0.15 wt. % to about 0.35 wt. % chromium.
18. The method of claim 17, further comprises providing a plurality of steel strips to be welded together, each of the steel strips including from about 1.20 wt. % to about 1.60 wt. % manganese.

## 17

19. The method of claim 17, further comprises providing a plurality of steel strips to be welded together, each of the plurality of steel strips including from about 0.15 wt. % to about 0.35 wt. % silicon.

20. The method of claim 17, further comprises providing a plurality of steel strips to be welded together, each of the plurality of steel strips including less than about 0.005 wt. % sulfur.

21. The method of claim 17, further comprises providing a plurality of steel strips to be welded together, each of the plurality of steel strips including from about 0.015 wt. % to about 0.070 wt. % aluminum.

22. The method of claim 17, further comprises providing a plurality of steel strips to be welded together, each of the plurality of steel strips including less than about 0.020 wt. % phosphorus.

23. A method of forming and heat treating a tube, the method comprising:

providing a plurality of steel strips to be welded together, each of the steel strips including from about 0.010 wt. % to about 0.025 wt. % titanium and from about 0.0010 wt. % to about 0.0025 wt. % of boron; welding the plurality of steel strips together end-to-end to form a plurality of end-to-end welded strips and longitudinally welding the plurality of end-to-end welded strips to form a tube having a first microstructure and comprising:  
 a first tube section with a substantially constant inner diameter, outer diameter, and wall thickness, said first portion of coiled tubing having a first microstructure; and  
 a second tube section with a wall thickness that is different than the wall thickness of the first tube section;  
 after forming the tube, performing a continuous and dynamic heat treatment process (CDHT) comprising a continuous quench and temper heat treatment along the tube, wherein heating rate is modified to compensate for the change in wall thickness from the first tube section to the second tube section, thereby resulting in a tube with a second microstructure comprising at least 80% tempered martensite across (a) the plurality of steel strips, (b) the plurality of end-to-end welds, and (c) the plurality of longitudinal welds, wherein the second microstructure is more homogeneous than the first microstructure; and  
 coiling the first portion of coiled tubing to form a coiled tube.

24. The method of claim 23, wherein the step of coiling the first portion of coiled tubing to form a coiled tube comprises coiling the first portion of coiled tubing on a spool.

25. The method of claim 23, further comprising:  
 after forming the first portion of coiled tubing, coiling the first portion of coiled tubing on a spool;  
 uncoiling the first portion of coiled tubing from the spool prior to performing the CDHT process;  
 performing the CDHT process; and  
 after performing the CDHT process, re-coiling the first portion of coiled tubing.

26. The method of claim 23, wherein the plurality of steel strips have a substantially uniform steel.

27. The method of claim 23, wherein the first portion of coiled tubing has a tempered martensite microstructure along substantially its entire length.

28. The method of claim 23, wherein performing the continuous quench and temper heat treatment comprises

## 18

translating the first portion of coiled tubing through a heat treatment system that performs heating action, cooling action, or both.

29. The method of claim 28, wherein translating the first portion of coiled tubing is at variable speeds.

30. The method of claim 23, wherein the performing a continuous quench and temper heat treatment comprises at least one quenching operation, intermediate operation, and tempering operation.

31. The method of claim 23, wherein at least one parameter of the continuous quench and temper heat treatment process is selected from a group consisting of temperature, soak time, heating rate, and cooling rate.

32. The method of claim 23, wherein at least one parameter of the continuous quench and temper heat treatment is selected from a group consisting of at least two of temperature, soak time, heating rate, and cooling rate.

33. The method of claim 23, wherein a yield strength of the first portion of coiled tubing is between 80 ksi and 140 ksi.

34. The method of claim 23, wherein the step of providing a plurality of steel strips to be welded together, comprises each of the steel strips including from about 1.30 wt. % to about 1.50 wt. % manganese.

35. The method of claim 23, further comprises providing a plurality of steel strips to be welded together, each of the plurality of steel strips including from about 0.15 wt. % to about 0.35 wt. % silicon.

36. The method of claim 23, further comprises providing a plurality of steel strips to be welded together, each of the plurality of steel strips including less than about 0.005 wt. % sulfur.

37. The method of claim 23, further comprises providing a plurality of steel strips to be welded together, each of the plurality of steel strips including from about 0.015 wt. % to about 0.070 wt. % aluminum.

38. The method of claim 23, further comprises providing a plurality of steel strips to be welded together, each of the plurality of steel strips including less than about 0.020 wt. % phosphorus.

39. The method of claim 23, further comprises providing a plurality of steel strips to be welded together, each of the steel strips including from about 0.15 wt. % to about 0.35 wt. % chromium.

40. The method of claim 39, further comprises providing a plurality of steel strips to be welded together, each of the steel strips including from about 1.20 wt. % to about 1.60 wt. % manganese.

41. The method of claim 39, further comprises providing a plurality of steel strips to be welded together, each of the plurality of steel strips including from about 0.15 wt. % to about 0.35 wt. % silicon.

42. The method of claim 39, further comprises providing a plurality of steel strips to be welded together, each of the plurality of steel strips including less than about 0.005 wt. % sulfur.

43. The method of claim 39, further comprises providing a plurality of steel strips to be welded together, each of the plurality of steel strips including from about 0.015 wt. % to about 0.070 wt. % aluminum.

44. The method of claim 39, further comprises providing a plurality of steel strips to be welded together, each of the plurality of steel strips including less than about 0.020 wt. % phosphorus.